# EUROPEAN PATENT APPLICATION

(11) **EP 4 678 774 A1**
(43) Date of publication of application: **14.01.2026**
(21) Application number: 24766783.5
(22) Date of filing: 13.02.2024
(51) Int. Cl.: C22C 38/00, C22C 38/54, C21D 8/10, C21D 9/08

(54) **STEEL MATERIAL SUITABLE FOR USE IN SOUR SERVICE ENVIRONMENT**

(30) Priority: 09.03.2023 JP 2023036280
(71) Applicant: NIPPON STEEL CORPORATION, Chiyoda-ku Tokyo 100-8071 (JP)
(72) Inventor: YOSHIDA, Shinji, Tokyo 100-8071 (JP); ARAI, Yuji, Tokyo 100-8071 (JP)
(74) Representative: Zimmermann & Partner Patentanwälte mbB
(86) International application number: PCT/JP2024/004747
(87) International publication number: WO 2024/185411

(57) **Abstract**

A steel material that has a high yield strength and has excellent fracture toughness in a low-temperature sour environment is provided. The steel material according to the present disclosure has the chemical composition described in the description and has a yield strength σ_{YS} of 758 MPa or more, and a content of Mo near prior-austenite grain boundaries γ_{Mo} in the steel material is 5.0% by mass or more. Further, when the yield strength σ_{YS} of the steel material according to the present disclosure is less than 862 MPa, Fnl defined by Formula (1) satisfies -300 or more, and when the yield strength σ_{YS} is 862 MPa or more, Fnl defined by Formula (1) satisfies -520 or more. $Fn 1 = 83 \times \left({γ}_{Mo}-{10}^{- 7}\times √ρ\right) - {σ}_{YS}$

Where, the content of Mo near prior-austenite grain boundaries in percent by mass is substituted for γ_{Mo} in Formula (1), a dislocation density in m⁻² is substituted for ρ in Formula (1), and the yield strength in MPa is substituted for σ_{YS} in Formula (1).

## Description

### TECHNICAL FIELD

The present disclosure relates to a steel material, and more particularly relates to a steel material suitable for use in a sour environment.

### BACKGROUND ART

Due to the deepening of oil wells and gas wells (hereunder, oil wells and gas wells are collectively referred to as simply "oil wells"), there is a demand to enhance the strength of oil-well steel materials that are typified by oil-well steel pipes. Specifically, oil-well steel materials of 80 ksi grade (yield strength is 80 to less than 95 ksi, that is, 552 to less than 655 MPa) and 95 ksi grade (yield strength is 95 to less than 110 ksi, that is, 655 to less than 758 MPa) oil-well steel pipes are being widely utilized, and recently requests are also starting to be made for oil-well steel pipes of 110 ksi grade (yield strength is 110 to less than 125 ksi, that is, 758 to less than 862 MPa), 125 ksi grade (yield strength is 125 to less than 140 ksi, that is, 862 to less than 965 MPa), and 140 ksi or more (yield strength is 140 ksi or more, that is, 965 MPa or more).

On the other hand, most deep wells are sour environments containing corrosive hydrogen sulfide. In the present description, the term "sour environment" means an acidified environment containing hydrogen sulfide. Note that, in some cases a sour environment may also contain carbon dioxide. Oil-well steel pipes for use in such sour environments are required to have not only high strength, but also to have sulfide stress cracking resistance (hereunder, referred to as "SSC resistance").

Technology for enhancing the SSC resistance of steel materials as typified by oil-well steel pipes is proposed in Japanese Patent Application Publication No. 2000-297344 (Patent Literature 1), Japanese Patent Application Publication No. 2001-271134 (Patent Literature 2), and International Application Publication No. WO2008/123422 (Patent Literature 3).

An oil-well steel disclosed in Patent Literature 1 contains, in mass%, C: 0.15 to 0.3%, Cr: 0.2 to 1.5%, Mo: 0.1 to 1%, V: 0.05 to 0.3%, and Nb: 0.003 to 0.1%. In this oil-well steel, the total amount of precipitating carbides is within the range of 1.5 to 4% by mass, the proportion that MC-type carbides occupy among the total amount of carbides is within the range of 5 to 45% by mass, and when the wall thickness of the product is taken as t (mm), the proportion of M₂₃C₆-type carbides is (200/t) or less in percent by mass. It is described in Patent Literature 1 that the aforementioned oil-well steel is excellent in SSC resistance.

A low-alloy steel material disclosed in Patent Literature 2 consists of, in mass%, C: 0.2 to 0.35%, Si: 0.05 to 0.5%, Mn: 0.1 to 1%, P: 0.025% or less, S: 0.01% or less, Cr: 0.1 to 1.2%, Mo: 0.1 to 1%, B: 0.0001 to 0.005%, Al: 0.005 to 0.1%, N: 0.01% or less, V: 0.05 to 0.5%, Ni: 0.1% or less, W: 1.0% or less, and O: 0.01% or less, with the balance being Fe and impurities, and satisfies the formula (0.03 ≤ Mo × V ≤0.3) and the formula (0.5 × Mo - V + GS/10 ≥1) and has a yield strength of 1060 MPa or more. Note that, "GS" in the formula represents the ASTM grain size number of prior-austenite grains. It is described in Patent Literature 2 that the aforementioned low-alloy steel material is excellent in SSC resistance.

A low-alloy steel disclosed in Patent Literature 3 consists of, in mass%, C: 0.10 to 0.20%, Si: 0.05 to 1.0%, Mn: 0.05 to 1.5%, Cr: 1.0 to 2.0%, Mo: 0.05 to 2.0%, Al: 0.10% or less, and Ti: 0.002 to 0.05%, with Ceq (= C + (Mn/6) + (Cr + Mo + V)/5) being 0.65 or more, and the balance being Fe and impurities. Among the impurities, the low-alloy steel contains P: 0.025% or less, S: 0.010% or less, N: 0.007% or less, and B: less than 0.0003%. In the low-alloy steel, the number density of M₂₃C₆-type precipitates having a grain size of 1 µm or more is 0.1 /mm² or less. It is described in Patent Literature 3 that in this low-alloy steel, the SSC resistance is enhanced.

### CITATION LIST

### PATENT LITERATURE

Patent Literature 1: Japanese Patent Application Publication No. 2000-297344
Patent Literature 2: Japanese Patent Application Publication No. 2001-271134
Patent Literature 3: International Application Publication No. WO2008/123422

### SUMMARY OF INVENTION

### TECHNICAL PROBLEM

In this connection, with respect to SSC resistance, in recent years attention is being focused on the ability to suppress the propagation of cracks formed in a steel material in a sour environment. There is a concern that when stress is applied to a steel material in which a minute flaw has been formed, the minute flaw will become the starting point of a crack and that the crack will propagate. On the other hand, it is considered that if propagation of cracks can be suppressed, a steel material will have excellent resistance to fracturing (that is, excellent fracture toughness). Therefore, there is a demand for oil-well steel materials which have high strength and also have excellent fracture toughness in a sour environment.

Furthermore, in recent years, deep wells beneath the surface of the sea are also being actively developed. For example, in so-called "deep-sea offshore oil fields" that are at a water depth of 2000 m or more, the water temperature is low. In addition, usually, there is a tendency for fracture toughness to more easily decrease as the temperature of the environment decreases. Therefore, demand has begun for oil-well steel materials, as represented by oil-well steel pipes, which have high strength and also have excellent fracture toughness even in a low-temperature sour environment.

In the aforementioned Patent Literatures 1 to 3, steel materials that have excellent SSC resistance are proposed. However, in the aforementioned Patent Literatures 1 to 3, no consideration is given to fracture toughness in a low-temperature sour environment.

An objective of the present disclosure is to provide a steel material which has high yield strength, and also has excellent fracture toughness in a low-temperature sour environment.

### SOLUTION TO PROBLEM

A steel material according to the present disclosure consists of, in mass%,
C: more than 0.20 to 0.60%,
Si: 0.05 to 2.00%,
Mn: 0.02 to 0.60%,
P: 0.025% or less,
S: 0.0100% or less,
Al: 0.005 to 0.100%,
Cr: 0.20 to 1.50%,
Mo: 0.35 to 1.50%,
V: 0.01 to 0.60%,
Ti: 0.002 to 0.050%,
B: 0.0001 to 0.0050%,
N: 0.0100% or less,
O: 0.0100% or less,
Nb: 0 to 0.030%,
Ca: 0 to 0.0100%,
Mg: 0 to 0.0100%,
Zr: 0 to 0.0100%,
rare earth metal: 0 to 0.0100%,
Co: 0 to 0.50%,
W: 0 to 0.50%,
Ni: 0 to 0.20%, and
Cu: 0 to 0.50%,
with the balance being Fe and impurities,
wherein:
   a yield strength σ_{YS} is 758 MPa or more;
   in the steel material, a content of Mo near prior-austenite grain boundaries γ_{Mo} is 5.0% by mass or more;
   in a case where the yield strength σ_{YS} is less than 862 MPa, Fn1 defined by Formula (1) satisfies -300 or more; and
   in a case where the yield strength σ_{YS} is 862 MPa or more, Fn1 defined by Formula (1) satisfies -520 or more; $Fn 1 = 83 \times \left({γ}_{Mo}-{10}^{- 7}\times √ρ\right) - {σ}_{YS}$
   where, the content of Mo near prior-austenite grain boundaries in percent by mass is substituted for γ_{Mo} in Formula (1), a dislocation density in m⁻² is substituted for ρ in Formula (1), and the yield strength in MPa is substituted for σ_{YS} in Formula (1).

### ADVANTAGEOUS EFFECTS OF INVENTION

The steel material according to the present disclosure has high yield strength, and has excellent fracture toughness in a low-temperature sour environment.

### BRIEF DESCRIPTION OF DRAWINGS

[FIG. 1] FIG. 1 is a view illustrating the relation between Fn1 (= 83 × (γ_{Mo} - 10⁻⁷ × √ρ) - σ_{YS}) and a fracture toughness value K_{1SSC} that is an index of fracture toughness in a low-temperature sour environment, in examples having a yield strength of 110 ksi grade (758 to less than 862 MPa) among the present examples.
[FIG. 2] FIG. 2 is a view illustrating the relation between Fn1 (= 83 × (γ_{Mo} - 10⁻⁷ × √ρ) - σ_{YS}) and a fracture toughness value K_{1SSC} that is an index of fracture toughness in a low-temperature sour environment, in examples having a yield strength of 125 ksi or more (862 MPa or more) among the present examples.
[FIG. 3] FIG. 3 is schematic diagram of an observation surface of a test specimen polished in order to determine a grain boundary Mo amount.
[FIG. 4] FIG. 4 is a schematic diagram of a measurement region 10 in which grain boundaries of prior-austenite grains were identified.
[FIG. 5] FIG. 5 is a schematic diagram illustrating the manner in which a thin film sample TP is prepared from the measurement region 10 illustrated in FIG. 4.
[FIG. 6] FIG. 6 is a perspective view of the thin film sample TP illustrated in FIG. 5.
[FIG. 7] FIG. 7 is a schematic diagram for describing the relation between an electron beam and a prior-austenite grain boundary GB in a thin film sample TP when performing TEM observation and elemental analysis by EDS.
[FIG. 8] FIG. 8 is a schematic diagram illustrating the relation between the irradiation direction of an electron beam EB when performing TEM observation and elemental analysis by EDS, a prior-austenite grain boundary GB of a surface 10 of a thin film sample TP, and an element concentration profile.
[FIG. 9] FIG. 9 is a view illustrating one example of the content of Mo on a line segment SL which is centered on a prior-austenite grain boundary GB and which is orthogonal to the prior-austenite grain boundary GB.
[FIG. 10] FIG. 10 is a schematic diagram for describing Formula (2).
[FIG. 11] FIG. 11 shows a side view and a cross-sectional view of a DCB test specimen used in a test (DCB test) for evaluating the fracture toughness of a steel material in a low-temperature sour environment in the present embodiment.
[FIG. 12] FIG. 12 is a perspective view of a wedge used in a test (DCB test) for evaluating the fracture toughness of a steel material in a low-temperature sour environment in the present embodiment.

### DESCRIPTION OF EMBODIMENTS

The present inventors carried out investigations and studies regarding methods for obtaining a steel material which has a high yield strength and also has excellent fracture toughness in a low-temperature sour environment, and obtained the following findings.

Specifically, the present inventors attempted to obtain a steel material having a yield strength of 758 MPa or more (110 ksi or more) as a high yield strength. Therefore, first, the present inventors conducted studies from the viewpoint of the chemical composition with respect to a steel material having a yield strength of 110 ksi or more and having excellent fracture toughness in a low-temperature sour environment. As a result, the present inventors considered that if a steel material consists of, in mass%, C: more than 0.20 to 0.60%, Si: 0.05 to 2.00%, Mn: 0.02 to 0.60%, P: 0.025% or less, S: 0.0100% or less, Al: 0.005 to 0.100%, Cr: 0.20 to 1.50%, Mo: 0.35 to 1.50%, V: 0.01 to 0.60%, Ti: 0.002 to 0.050%, B: 0.0001 to 0.0050%, N: 0.0100% or less, O: 0.0100% or less, Nb: 0 to 0.030%, Ca: 0 to 0.0100%, Mg: 0 to 0.0100%, Zr: 0 to 0.0100%, rare earth metal: 0 to 0.0100%, Co: 0 to 0.50%, W: 0 to 0.50%, Ni: 0 to 0.20%, and Cu: 0 to 0.50%, with the balance being Fe and impurities, there is a possibility of obtaining a steel material which has a yield strength of 110 ksi or more and which has excellent fracture toughness in a low-temperature sour environment.

Next, the present inventors investigated various techniques for increasing fracture toughness in a low-temperature sour environment with respect to a steel material which has the chemical composition described above and has a yield strength of 110 ksi or more. As a result, it was revealed that in a steel material having the aforementioned chemical composition and yield strength, in a low-temperature sour environment, a decrease in toughness at prior-austenite grain boundaries in the steel material easily occurs, and propagation of cracks easily proceeds along prior-austenite grain boundaries in the steel material. That is, in a steel material having the aforementioned chemical composition and yield strength, if prior-austenite grain boundaries can be strengthened, there is a possibility that excellent fracture toughness will be obtained. Hereunder, in the present description, prior-austenite grains are also referred to as "prior-y grains".

Therefore, the present inventors focused their attention on molybdenum (Mo) as an element that contributes to strengthening of prior-y grain boundaries. If Mo concentrates at prior-y grain boundaries, the prior-y grain boundaries can be strengthened and there is a possibility that the propagation of cracks can be suppressed even in a low-temperature sour environment. As a result, there is a possibility that excellent fracture toughness will be obtained in a low-temperature sour environment. As a result of detailed studies conducted by the present inventors, it was revealed that in a steel material having the chemical composition described above and a yield strength of 110 ksi or more, if a content of Mo near prior-y grain boundaries γ_{Mo} is 5.0% by mass or more, there is a possibility that excellent fracture toughness can be obtained. Hereinafter, in the present description, the content of Mo near prior-y grain boundaries γ_{Mo} is also referred to as "grain boundary Mo amount γ_{Mo}".

On the other hand, even when steel materials had the chemical composition and yield strength described above, and the grain boundary Mo amount γ_{Mo} in the steel materials was 5.0% by mass or more, in some cases excellent fracture toughness was not stably obtained in a low-temperature sour environment. Therefore the present inventors carried out more detailed studies regarding factors which cause the fracture toughness to decrease in the aforementioned steel materials. As a result, it was revealed that in a steel material having the chemical composition and yield strength described above, the fracture toughness in a low-temperature sour environment is influenced by a dislocation density ρ in the steel material, the yield strength σ_{YS} of the steel material, and the grain boundary Mo amount γ_{Mo}.

Here, let Fn1 be defined as Fn1 = 83 × (γ_{Mo} - 10⁻⁷ × √ρ) - σ_{YS}. Fn1 is an index of fracture toughness in a low-temperature sour environment. Hereunder, a case where the yield strength σ_{YS} is less than 862 MPa (758 to less than 862 MPa), and a case where the yield strength σ_{YS} is 862 MPa or more will each be specifically described using separate drawings.

FIG. 1 is a view illustrating the relation between Fn1 (= 83 × (γ_{Mo} - 10⁻⁷ × √ρ) - σ_{YS}) and a fracture toughness value K_{1SSC} that is an index of fracture toughness in a low-temperature sour environment, in examples which had a yield strength of 110 ksi grade (758 to less than 862 MPa) among the present examples. FIG. 1 was prepared using examples which, among examples to be described later, satisfied the chemical composition described above and had a yield strength σ_{YS} of 110 ksi grade, and in which the grain boundary Mo amount γ_{Mo} was 5.0% by mass or more. Note that, the yield strength σ_{YS}, the grain boundary Mo amount γ_{Mo}, the dislocation density ρ, and the fracture toughness value K_{1SSC} were determined by methods which are described later.

Referring to FIG. 1, it can be confirmed that in steel materials having the chemical composition described above, a yield strength of 110 ksi grade, and a grain boundary Mo amount γ_{Mo} of 5.0% by mass or more, when Fn1 is -300 or more, the fracture toughness value K_{1SSC} in a low-temperature sour environment is 29.5 MPa√m or more, and excellent fracture toughness is stably exhibited. On the other hand, in the aforementioned steel materials, when Fn1 is less than -300, the fracture toughness value K_{1SSC} in a low-temperature sour environment is less than 29.5 MPa√m, and excellent fracture toughness is not exhibited. Accordingly, the steel material according to the present embodiment has the chemical composition described above and a grain boundary Mo amount γ_{Mo} of 5.0% by mass or more, and when the yield strength σ_{YS} is 758 to less than 862 MPa, Fn1 is -300 or more.

Further, FIG. 2 is a view illustrating the relation between Fn1 (= 83 × (γ_{Mo} - 10⁻⁷ × √ρ) - σ_{YS}) and a fracture toughness value K_{1SSC} that is an index of fracture toughness in a low-temperature sour environment, in examples having a yield strength of 125 ksi or more (862 MPa or more) among the present examples. FIG. 2 was prepared using examples which, among examples to be described later, satisfied the chemical composition described above and had a yield strength σ_{YS} of 125 ksi or more, and in which the grain boundary Mo amount γ_{Mo} was 5.0% by mass or more. Note that, the yield strength σ_{YS}, the grain boundary Mo amount γ_{Mo}, the dislocation density ρ, and the fracture toughness value K_{1SSC} were determined by methods which are described later.

Referring to FIG. 2, it can be confirmed that in steel materials having the chemical composition described above, a yield strength of 125 ksi or more, and a grain boundary Mo amount γ_{Mo} of 5.0% by mass or more, when Fn1 is -520 or more, the fracture toughness value K_{1SSC} in a low-temperature sour environment is 24.1 MPa√m or more, and excellent fracture toughness is stably exhibited. On the other hand, in the aforementioned steel materials, when Fn1 is less than -520, the fracture toughness value K_{1SSC} in a low-temperature sour environment is less than 24.1 MPa√m, and excellent fracture toughness is not exhibited. Accordingly, the steel material according to the present embodiment has the chemical composition described above and a grain boundary Mo amount γ_{Mo} of 5.0% by mass or more, and when the yield strength σ_{YS} is 862 MPa or more, Fn1 is -520 or more.

Note that, the reason why the fracture toughness in a low-temperature sour environment can be increased by adjusting Fn1 in a steel material having the chemical composition, the yield strength σ_{YS}, and the grain boundary Mo amount γ_{Mo} that are described above has not been clarified in detail. However, the present inventors surmise that the reason is as follows. As described above, Fn1 defines the relation between the yield strength σ_{YS}, the grain boundary Mo amount γ_{Mo}, and the dislocation density ρ. Here, it is considered that while, on the one hand, dislocations increase the yield strength σ_{YS} of the steel material, on the other hand, dislocations occlude hydrogen. Therefore, there is a risk that if the dislocation density ρ is too high, hydrogen occluded by the dislocations will tend to stay at prior-γ grain boundaries, and consequently the prior-y grain boundaries will easily become brittle. That is, there is a possibility that if the dislocation density ρ can be lowered, the amount of hydrogen that stays at prior-y grain boundaries can be reduced and the prior-y grain boundaries can be strengthened. However, as described above, the dislocation density ρ contributes to increasing the yield strength σ_{YS}. Therefore, there is a possibility that in a steel material having the chemical composition described above, the fracture toughness in a low-temperature sour environment can be increased by controlling the relation between the yield strength σ_{YS}, the grain boundary Mo amount γ_{Mo}, and the dislocation density ρ, rather than simply lowering the dislocation density ρ.

The present inventors surmise that in the steel material according to the present embodiment, high strength as well as excellent fracture toughness in a low-temperature sour environment are obtained by the mechanism described above. Note that, it is also possible that by adjusting Fn1 in a steel material having the chemical composition, the yield strength σ_{YS}, and the grain boundary Mo amount γ_{Mo} which are described above, the fracture toughness in a low-temperature sour environment can be increased by a mechanism other than the mechanism described above. However, the fact that in a steel material having the chemical composition, the yield strength σ_{YS}, and the grain boundary Mo amount γ_{Mo} which are described above, the fracture toughness in a low-temperature sour environment can be increased by adjusting Fn1 has been demonstrated by Examples that are described later.

The gist of the steel material according to the present embodiment, which has been completed based on the findings described above, is as follows.
[1] A steel material consisting of, in mass%,
   C: more than 0.20 to 0.60%,
   Si: 0.05 to 2.00%,
   Mn: 0.02 to 0.60%,
   P: 0.025% or less,
   S: 0.0100% or less,
   Al: 0.005 to 0.100%,
   Cr: 0.20 to 1.50%,
   Mo: 0.35 to 1.50%,
   V: 0.01 to 0.60%,
   Ti: 0.002 to 0.050%,
   B: 0.0001 to 0.0050%,
   N: 0.0100% or less,
   O: 0.0100% or less,
   Nb: 0 to 0.030%,
   Ca: 0 to 0.0100%,
   Mg: 0 to 0.0100%,
   Zr: 0 to 0.0100%,
   rare earth metal: 0 to 0.0100%,
   Co: 0 to 0.50%,
   W: 0 to 0.50%,
   Ni: 0 to 0.20%, and
   Cu: 0 to 0.50%,
   with the balance being Fe and impurities,
   wherein:
      a yield strength σ_{YS} is 758 MPa or more;
      in the steel material, a content of Mo near prior-austenite grain boundaries γ_{Mo} is 5.0% by mass or more;
      in a case where the yield strength σ_{YS} is less than 862 MPa, Fn1 defined by Formula (1) satisfies -300 or more; and
      in a case where the yield strength σ_{YS} is 862 MPa or more, Fn1 defined by Formula (1) satisfies -520 or more; $Fn 1 = 83 \times \left({γ}_{Mo}-{10}^{- 7}\times √ρ\right) - {σ}_{YS}$
      where, the content of Mo near prior-austenite grain boundaries in percent by mass is substituted for γ_{Mo} in Formula (1), a dislocation density in m⁻² is substituted for ρ in Formula (1), and the yield strength in MPa is substituted for σ_{YS} in Formula (1).
[2] The steel material according to [1], containing one or more elements selected from a group consisting of:
   Nb: 0.001 to 0.030%,
   Ca: 0.0001 to 0.0100%,
   Mg: 0.0001 to 0.0100%,
   Zr: 0.0001 to 0.0100%,
   rare earth metal: 0.0001 to 0.0100%,
   Co: 0.01 to 0.50%,
   W: 0.01 to 0.50%,
   Ni: 0.01 to 0.20%, and
   Cu: 0.01 to 0.50%.
[3] The steel material according to [1] or [2], wherein:
   the steel material is an oil-well steel pipe.

Note that, the shape of the steel material according to the present embodiment is not particularly limited. The steel material according to the present embodiment may be a steel pipe, may be a round steel bar (solid material), or may be a steel plate. Note that, the term "round steel bar" refers to a steel bar in which a cross section in a direction perpendicular to the axial direction is a circular shape. Further, the steel pipe may be a seamless steel pipe, or may be a welded steel pipe.

Hereunder, the steel material according to the present embodiment is described in detail.

### [Chemical composition]

The chemical composition of the steel material according to the present embodiment contains the following elements. The symbol "%" in relation to an element means mass percent unless otherwise stated.

### C: more than 0.20 to 0.60%

Carbon (C) increases hardenability of the steel material and increases the strength of the steel material. C also promotes spheroidization of carbides during tempering in the production process, and thereby enhances the SSC resistance of the steel material. If carbides are dispersed, the strength of the steel material will increase further. If the content of C is too low, even if the contents of other elements are within the range of the present embodiment, the aforementioned advantageous effects will not be sufficiently obtained. On the other hand, if the content of C is too high, even if the contents of other elements are within the range of the present embodiment, there will be too many carbides produced and the toughness of the steel material will decrease. In addition, if the content of C is too high, in some cases quench cracking will easily occur during quenching in the production process. Therefore, the content of C is to be more than 0.20 to 0.60%. A preferable lower limit of the content of C is 0.22%, more preferably is 0.24%, and further preferably is 0.25%. A preferable upper limit of the content of C is 0.55%, more preferably is 0.50%, and further preferably is 0.45%.

### Si: 0.05 to 2.00%

Silicon (Si) deoxidizes the steel. If the Si content is too low, the aforementioned advantageous effect will not be sufficiently obtained even if the contents of other elements are within the range of the present embodiment. On the other hand, if the content of Si is too high, even if the contents of other elements are within the range of the present embodiment, the SSC resistance of the steel material will decrease. Therefore, the content of Si is to be 0.05 to 2.00%. A preferable lower limit of the content of Si is 0.15%, and more preferably is 0.20%. A preferable upper limit of the content of Si is 1.80%, more preferably is 1.60%, further preferably is 1.50%, and further preferably is 1.40%.

### Mn: 0.02 to 0.60%

Manganese (Mn) deoxidizes the steel. Mn also increases hardenability of the steel material and increases the strength of the steel material. If the content of Mn is too low, even if the contents of other elements are within the range of the present embodiment, the aforementioned advantageous effects will not be sufficiently obtained. On the other hand, if the content of Mn is too high, even if the contents of other elements are within the range of the present embodiment, Mn will segregate to grain boundaries together with impurities such as P and S, and the fracture toughness of the steel material in a low-temperature sour environment will decrease. Therefore, the content of Mn is to be 0.02 to 0.60%. A preferable lower limit of the content of Mn is 0.03%, more preferably is 0.04%, and further preferably is 0.06%. A preferable upper limit of the content of Mn is 0.55%, more preferably is 0.50%, and further preferably is 0.45%.

### P: 0.025% or less

Phosphorus (P) is an impurity. That is, the lower limit of the content of P is more than 0%. If the content of P is too high, even if the contents of other elements are within the range of the present embodiment, P will segregate to grain boundaries and the fracture toughness of the steel material in a low-temperature sour environment will decrease. Therefore, the content of P is to be 0.025% or less. A preferable upper limit of the content of P is 0.020%, and more preferably is 0.015%. The content of P is preferably as low as possible. However, extremely reducing the content of P will greatly increase the production cost. Therefore, when taking industrial production into consideration, a preferable lower limit of the content of P is 0.001 %, more preferably is 0.002%, and further preferably is 0.003%.

### S: 0.0100% or less

Sulfur (S) is an impurity. That is, the lower limit of the content of S is more than 0%. If the content of S is too high, even if the contents of other elements are within the range of the present embodiment, S will segregate to grain boundaries and the SSC resistance of the steel material will decrease. Therefore, the content of S is to be 0.0100% or less. A preferable upper limit of the content of S is 0.0075%, more preferably is 0.0050%, and further preferably is 0.0030%. The content of S is preferably as low as possible. However, extremely reducing the content of S will greatly increase the production cost. Therefore, when taking industrial production into consideration, a preferable lower limit of the content of S is 0.0001%, more preferably is 0.0002%, and further preferably is 0.0003%.

### Al: 0.005 to 0.100%

Aluminum (Al) deoxidizes the steel. If the content of Al is too low, the aforementioned advantageous effect will not be sufficiently obtained even if the contents of other elements are within the range of the present embodiment. As a result, the SSC resistance of the steel material will decrease. On the other hand, if the content of Al is too high, even if the contents of other elements are within the range of the present embodiment, coarse oxide-based inclusions will form and the SSC resistance of the steel material will decrease. Therefore, the content of Al is to be 0.005 to 0.100%. A preferable lower limit of the content of Al is 0.015%, and more preferably is 0.020%. A preferable upper limit of the content of Al is 0.080%, and more preferably is 0.060%. As used in the present description, the content of "Al" means the content of "acid-soluble Al", that is, "sol. Al".

### Cr: 0.20 to 1.50%

Chromium (Cr) increases hardenability of the steel material and increases the strength of the steel material. Cr also increases the temper softening resistance of the steel material and thereby enables high-temperature tempering. As a result, the fracture toughness of the steel material in a low-temperature sour environment increases. If the content of Cr is too low, the aforementioned advantageous effects will not be sufficiently obtained even if the contents of other elements are within the range of the present embodiment. On the other hand, if the content of Cr is too high, even if the contents of other elements are within the range of the present embodiment, the SSC resistance of the steel material will decrease. Therefore, the content of Cr is to be 0.20 to 1.50%. A preferable lower limit of the content of Cr is 0.25%, more preferably is 0.30%, further preferably is 0.35%, and further preferably is 0.40%. A preferable upper limit of the content of Cr is 1.40%, and more preferably is 1.30%.

### Mo: 0.35 to 1.50%

Molybdenum (Mo) increases hardenability of the steel material and increases the strength of the steel material. Mo also increases the grain boundary Mo amount γ_{Mo}, and increases the fracture toughness of the steel material in a low-temperature sour environment. If the content of Mo is too low, the aforementioned advantageous effects will not be sufficiently obtained even if the contents of other elements are within the range of the present embodiment. On the other hand, if the content of Mo is too high, the aforementioned advantageous effects will be saturated. Therefore, the content of Mo is to be 0.35 to 1.50%. A preferable lower limit of the content of Mo is 0.40%, more preferably is 0.45%, and further preferably is 0.50%. A preferable upper limit of the content of Mo is 1.40%, more preferably is 1.30%, and further preferably is 1.25%.

### V: 0.01 to 0.60%

Vanadium (V) combines with C or N to form carbides, nitrides, or carbo-nitrides (hereunder, also referred to as "carbo-nitrides and the like"), and refines the grains of the steel material by the pinning effect. As a result, the fracture toughness of the steel material in a low-temperature sour environment increases. V also forms fine carbides during tempering and thereby increases the temper softening resistance of the steel material and increases the strength of the steel material. If the content of V is too low, the aforementioned advantageous effects will not be sufficiently obtained even if the contents of other elements are within the range of the present embodiment. On the other hand, if the content of V is too high, the toughness of the steel material will decrease even if the contents of other elements are within the range of the present embodiment. Therefore, the content of V is to be 0.01 to 0.60%. A preferable lower limit of the content of V is 0.02%, more preferably is 0.04%, and further preferably is 0.06%. A preferable upper limit of the content of V is 0.40%, more preferably is 0.30%, further preferably is 0.25%, and further preferably is 0.20%.

### Ti: 0.002 to 0.050%

Titanium (Ti) combines with N to form nitrides, and refines the grains of the steel material by the pinning effect. As a result, the fracture toughness of the steel material in a low-temperature sour environment increases. If the content of Ti is too low, the aforementioned advantageous effect will not be sufficiently obtained even if the contents of other elements are within the range of the present embodiment. On the other hand, if the content of Ti is too high, even if the contents of other elements are within the range of the present embodiment, Ti nitrides will coarsen and the SSC resistance of the steel material will decrease. Therefore, the content of Ti is to be 0.002 to 0.050%. A preferable lower limit of the content of Ti is 0.003%, and more preferably is 0.005%. A preferable upper limit of the content of Ti is 0.030%, and more preferably is 0.020%.

### B: 0.0001 to 0.0050%

Boron (B) dissolves in the steel and thereby increases hardenability of the steel material and increases the strength of the steel material. If the content of B is too low, the aforementioned advantageous effect will not be sufficiently obtained even if the contents of other elements are within the range of the present embodiment. On the other hand, if the content of B is too high, even if the contents of other elements are within the range of the present embodiment, coarse nitrides will form and the SSC resistance of the steel material will decrease. Therefore, the content of B is to be 0.0001 to 0.0050%. A preferable lower limit of the content of B is 0.0003%, and more preferably is 0.0007%. A preferable upper limit of the content of B is 0.0030%, more preferably is 0.0025%, further preferably is 0.0020%, and further preferably is 0.0015%.

### N: 0.0100% or less

Nitrogen (N) is unavoidably contained. That is, the lower limit of the content of N is more than 0%. N combines with Ti to form nitrides, and refines grains of the steel material by the pinning effect. As a result, the fracture toughness of the steel material in a low-temperature sour environment increases. However, if the content of N is too high, even if the contents of other elements are within the range of the present embodiment, coarse nitrides will be formed and the fracture toughness of the steel material in a low-temperature sour environment will, on the contrary, decrease. Therefore, the content of N is to be 0.0100% or less. A preferable upper limit of the content of N is 0.0060%, more preferably is 0.0050%, and further preferably is 0.0045%. A preferable lower limit of the content of N for more effectively obtaining the aforementioned advantageous effect is 0.0005%, more preferably is 0.0010%, further preferably is 0.0015%, and further preferably is 0.0020%.

### O: 0.0100% or less

Oxygen (O) is an impurity. That is, the lower limit of the content of O is more than 0%. If the content of O is too high, even if the contents of other elements are within the range of the present embodiment, coarse oxides will form and the low-temperature toughness and SSC resistance of the steel material will decrease. Therefore, the content of O is to be 0.0100% or less. A preferable upper limit of the content of O is 0.0050%, more preferably is 0.0030%, and further preferably is 0.0020%. The content of O is preferably as low as possible. However, extremely reducing the content of O will greatly increase the production cost. Therefore, when taking industrial production into consideration, a preferable lower limit of the content of O is 0.0001%, more preferably is 0.0002%, and further preferably is 0.0003%.

The balance of the chemical composition of the steel material according to the present embodiment is Fe and impurities. Here, the term "impurities" refers to substances which, when industrially producing the steel material, are mixed in from ore or scrap that is used as the raw material or from the production environment or the like, and which are allowed within a range that does not adversely affect the steel material according to the present embodiment.

### [Optional elements]

The chemical composition of the steel material described above may further contain Nb in lieu of a part of Fe.

### Nb: 0 to 0.030%

Niobium (Nb) is an optional element, and does not have to be contained. That is, the content of Nb may be 0%. When contained, Nb forms carbo-nitrides and the like, and refines the grains of the steel material by the pinning effect. As a result, the fracture toughness of the steel material in a low-temperature sour environment increases. Nb also forms fine carbides during tempering and thereby increases the temper softening resistance of the steel material and increases the strength of the steel material. If even a small amount of Nb is contained, the aforementioned advantageous effects will be obtained to a certain extent. However, if the content of Nb is too high, even if the contents of other elements are within the range of the present embodiment, carbo-nitrides and the like will be excessively formed and the SSC resistance of the steel material will decrease. Therefore, the content of Nb is to be 0 to 0.030%. A preferable lower limit of the content of Nb is more than 0%, more preferably is 0.001%, further preferably is 0.002%, further preferably is 0.003%, further preferably is 0.005%, and further preferably is 0.007%. A preferable upper limit of the content of Nb is 0.025%, and more preferably is 0.020%.

The chemical composition of the steel material described above may further contain one or more elements selected from the group consisting of Ca, Mg, Zr and rare earth metal in lieu of a part of Fe. Each of these elements is an optional element, and render S in the steel material harmless by forming sulfides. As a result, these elements increase the SSC resistance of the steel material.

### Ca: 0 to 0.0100%

Calcium (Ca) is an optional element, and does not have to be contained. That is, the content of Ca may be 0%. When contained, Ca renders S in the steel material harmless by forming sulfides, and thereby increases the SSC resistance of the steel material. If even a small amount of Ca is contained, the aforementioned effect will be obtained to a certain extent. However, if the content of Ca is too high, even if the contents of other elements are within the range of the present embodiment, oxides in the steel material will coarsen and the SSC resistance of the steel material will, on the contrary, decrease. Therefore, the content of Ca is to be 0 to 0.0100%. A preferable lower limit of the content of Ca is more than 0%, more preferably is 0.0001%, further preferably is 0.0003%, further preferably is 0.0006%, and further preferably is 0.0010%. A preferable upper limit of the content of Ca is 0.0040%, more preferably is 0.0030%, further preferably is 0.0025%, and further preferably is 0.0020%.

### Mg: 0 to 0.0100%

Magnesium (Mg) is an optional element, and does not have to be contained. That is, the content of Mg may be 0%. When contained, Mg renders S in the steel material harmless by forming sulfides, and thereby increases the SSC resistance of the steel material. If even a small amount of Mg is contained, the aforementioned effect will be obtained to a certain extent. However, if the content of Mg is too high, even if the contents of other elements are within the range of the present embodiment, oxides in the steel material will coarsen and the SSC resistance of the steel material will decrease. Therefore, the content of Mg is to be 0 to 0.0100%. A preferable lower limit of the content of Mg is more than 0%, more preferably is 0.0001%, further preferably is 0.0003%, further preferably is 0.0006%, and further preferably is 0.0010%. A preferable upper limit of the content of Mg is 0.0040%, more preferably is 0.0030%, further preferably is 0.0025%, and further preferably is 0.0020%.

### Zr: 0 to 0.0100%

Zirconium (Zr) is an optional element, and does not have to be contained. That is, the content of Zr may be 0%. When contained, Zr renders S in the steel material harmless by forming sulfides, and thereby increases the SSC resistance of the steel material. If even a small amount of Zr is contained, the aforementioned effect will be obtained to a certain extent. However, if the content of Zr is too high, even if the contents of other elements are within the range of the present embodiment, oxides in the steel material will coarsen and the SSC resistance of the steel material will decrease. Therefore, the content of Zr is to be 0 to 0.0100%. A preferable lower limit of the content of Zr is more than 0%, more preferably is 0.0001%, further preferably is 0.0003%, further preferably is 0.0006%, and further preferably is 0.0010%. A preferable upper limit of the content of Zr is 0.0040%, more preferably is 0.0030%, further preferably is 0.0025%, and further preferably is 0.0020%.

### Rare earth metal (REM): 0 to 0.0100%

Rare earth metal (REM) is an optional element, and does not have to be contained. That is, the content of REM may be 0%. When contained, REM renders S in the steel material harmless by forming sulfides, and thereby increases the SSC resistance of the steel material. REM also combines with P in the steel material and thereby suppresses segregation of P to the grain boundaries. Therefore, a decrease in the SSC resistance of the steel material attributable to segregation of P is suppressed. If even a small amount of REM is contained, the aforementioned advantageous effects will be obtained to a certain extent even if the contents of other elements are within the range of the present embodiment. However, if the content of REM is too high, even if the contents of other elements are within the range of the present embodiment, oxides in the steel material will coarsen and the SSC resistance of the steel material will decrease. Therefore, the content of REM is to be 0 to 0.0100%. A preferable lower limit of the content of REM is more than 0%, more preferably is 0.0001%, further preferably is 0.0003%, and further preferably is 0.0006%. A preferable upper limit of the content of REM is 0.0040%, more preferably is 0.0030%, and further preferably is 0.0025%.

Note that, in the present description, the term "REM" means one or more types of element selected from the group consisting of scandium (Sc) which is the element with atomic number 21, yttrium (Y) which is the element with atomic number 39, and the elements from lanthanum (La) with atomic number 57 to lutetium (Lu) with atomic number 71 that are lanthanoids. In the present description, the term "content of REM" refers to the total content of these elements.

The chemical composition of the steel material described above may further contain one or more elements selected from the group consisting of Co and W in lieu of a part of Fe. Each of these elements is an optional element that forms a protective corrosion coating in a sour environment and suppresses penetration of hydrogen into the steel material. By this means, each of these elements increases the SSC resistance of the steel material.

### Co: 0 to 0.50%

Cobalt (Co) is an optional element, and does not have to be contained. That is, the content of Co may be 0%. When contained, Co forms a protective corrosion coating in a sour environment and suppresses penetration of hydrogen into the steel material. As a result, the SSC resistance of the steel material increases. If even a small amount of Co is contained, the aforementioned effect will be obtained to a certain extent. However, if the content of Co is too high, even if the contents of other elements are within the range of the present embodiment, hardenability of the steel material will decrease, and the strength of the steel material will decrease. Therefore, the content of Co is to be 0 to 0.50%. A preferable lower limit of the content of Co is more than 0%, more preferably is 0.01%, further preferably is 0.02%, further preferably is 0.03%, and further preferably is 0.05%. A preferable upper limit of the content of Co is 0.45%, and more preferably is 0.40%.

### W: 0 to 0.50%

Tungsten (W) is an optional element, and does not have to be contained. That is, the content of W may be 0%. When contained, W forms a protective corrosion coating in a sour environment and suppresses penetration of hydrogen into the steel material. As a result, the SSC resistance of the steel material increases. If even a small amount of W is contained, the aforementioned effect will be obtained to a certain extent. However, if the content of W is too high, even if the contents of other elements are within the range of the present embodiment, coarse carbides will form in the steel material, and the low-temperature toughness and SSC resistance of the steel material will decrease. Therefore, the content of W is to be 0 to 0.50%. A preferable lower limit of the content of W is more than 0%, more preferably is 0.01%, further preferably is 0.02%, further preferably is 0.03%, and further preferably is 0.05%. A preferable upper limit of the content of W is 0.45%, and more preferably is 0.40%.

The chemical composition of the steel material described above may further contain one or more types of element selected from the group consisting of Ni and Cu in lieu of a part of Fe. Each of these elements is an optional element, and each element increases hardenability of the steel material.

### Ni: 0 to 0.20%

Nickel (Ni) is an optional element, and does not have to be contained. That is, the content of Ni may be 0%. When contained, Ni increases hardenability of the steel material and increases the strength of the steel material. Ni also dissolves in the steel and increases the low-temperature toughness of the steel material. If even a small amount of Ni is contained, these advantageous effects will be obtained to a certain extent. However, if the content of Ni is too high, even if the contents of other elements are within the range of the present embodiment, local corrosion will be promoted and the SSC resistance of the steel material will decrease. Therefore, the content of Ni is to be 0 to 0.20%. A preferable lower limit of the content of Ni is more than 0%, more preferably is 0.01%, and further preferably is 0.02%. A preferable upper limit of the content of Ni is 0.15%, more preferably is 0.10%, further preferably is 0.09%, further preferably is 0.08%, and further preferably is 0.06%.

### Cu: 0 to 0.50%

Copper (Cu) is an optional element, and does not have to be contained. That is, the content of Cu may be 0%. When contained, Cu increases hardenability of the steel material and increases the strength of the steel material. If even a small amount of Cu is contained, the aforementioned effect will be obtained to a certain extent. However, if the content of Cu is too high, even if the contents of other elements are within the range of the present embodiment, the hardenability of the steel material will be too high and the SSC resistance of the steel material will decrease. Therefore, the content of Cu is to be 0 to 0.50%. A preferable lower limit of the content of Cu is more than 0%, more preferably is 0.01%, further preferably is 0.02%, and further preferably is 0.05%. A preferable upper limit of the content of Cu is 0.35%, and more preferably is 0.25%.

### [Yield strength σ_{YS}]

A yield strength σ_{YS} of the steel material according to the present embodiment is 758 MPa or more (110 ksi or more). As used in the present description, the term "yield strength" means 0.2% offset proof stress obtained in a tensile test carried out in conformity with ASTM E8/E8M (2021). Note that, an upper limit of the yield strength of the steel material according to the present embodiment is not particularly limited. However, it has been demonstrated by Examples that are described later that at least when the yield strength is within a range of 758 to 965 MPa, the steel material according to the present embodiment has excellent fracture toughness in a low-temperature sour environment. Therefore, the range of the yield strength of the steel material according to the present embodiment includes at least 758 to 965 MPa (110 to 140 ksi). That is, the range of the yield strength of the steel material according to the present embodiment includes at least 758 to less than 862 MPa (110 ksi grade) and 862 to 965 MPa (125 ksi grade).

The yield strength of the steel material according to the present embodiment can be determined by the following method. Specifically, a tensile test is performed in conformity with ASTM E8/E8M (2021). A round bar specimen is prepared from the steel material according to the present embodiment. If the steel material is a steel plate, the round bar specimen is prepared from the center portion of the thickness. In this case, the axial direction of the round bar specimen is to be made a direction that is parallel to the rolling elongation direction of the steel plate. If the steel material is a steel pipe, the round bar specimen is prepared from the center portion of the wall thickness. In this case, the axial direction of the round bar specimen is to be made a direction that is parallel to the axial direction of the steel pipe. If the steel material is a round steel bar, the round bar specimen is prepared from an R/2 position. In this case, the axial direction of the round bar specimen is to be made a direction that is parallel to the axial direction of the round steel bar. Note that, in the present description, the term "R/2 position" means the center position of a radius R in a cross section perpendicular to the axial direction of the round steel bar. Regarding the size of the round bar specimen, for example, the round bar specimen has a parallel portion diameter of 4 mm and a gage length of 16 mm. A tensile test is carried out in the atmosphere at normal temperature (25°C) using the round bar specimen, and the obtained 0.2% offset proof stress is defined as the yield strength (MPa). Note that, a value obtained by rounding off decimals of the obtained numerical value is adopted as the yield strength (MPa) in the present embodiment.

### [Grain boundary Mo amount γ_{Mo}]

A grain boundary Mo amount γ_{Mo} of the steel material according to the present embodiment is 5.0% by mass or more. As described above, in the present description, the term "grain boundary Mo amount γ_{Mo}" means the content of Mo near prior-austenite grain boundaries. In the present embodiment, the content of Mo near prior-austenite grain boundaries γ_{Mo} (grain boundary Mo amount γ_{Mo}) is defined as follows.

In the steel material according to the present embodiment, when:
one endpoint of a line segment SL having a length of 10 nm which is centered on a grain boundaries of prior-austenite grains and which is orthogonal to the grain boundaries is defined as "E1", and the other endpoint is defined as "E2",
at respective measurement points located at a pitch of 0.2 nm from the endpoint E1 to the endpoint E2 of the line segment SL, the content of Mo (mass%) at the respective measurement points on the line segment SL is determined by elemental analysis by energy dispersive X-ray spectrometry, and
on the line segment SL:
   a measurement point at which the content of Mo is maximum on the line segment SL is defined as "Mo peak measurement point",
   a region having a width of 2.0 nm which is centered on the Mo peak measurement point is defined as "Mo concentrated region",
   a region between the endpoint E1 and the Mo concentrated region is defined as "first Mo intra-grain region",
   a region between the endpoint E2 and the Mo concentrated region is defined as "second Mo intra-grain region",
   an arithmetic average value of the contents of Mo at all of the measurement points within the first Mo intra-grain region is defined as "γ_{Mo1} (mass%)", and
   an arithmetic average value of the contents of Mo at all of the measurement points within the second Mo intra-grain region is defined as "γ_{Mo2} (mass%)",
   the grain boundary Mo amount γ_{Mo} is defined by the following Formula (2). γMo = {(sum total of contents of Mo at all of the measurement points on the line segment SL × 0.2) - γMo1 × (distance between the endpoint E1 and the Mo peak measurement point) - γMo2 × (distance between the endpoint E2 and the Mo peak measurement point) }/0.8 + (γMo1 + γMo2)/2

More specifically, in the present embodiment, the grain boundary Mo amount γ_{Mo} can be determined by the following method. First, a test specimen for measuring the grain boundary Mo amount γ_{Mo} is prepared from the steel material according to the present embodiment. Specifically, a test specimen is prepared in which a surface perpendicular to a C direction of the steel material is made the observation surface. That is, the observation surface of the test specimen includes an L direction and a T direction. Here, if the steel material is a steel plate, the rolling elongation direction is defined as "L direction", the thickness direction is defined as "T direction", and the plate width direction is defined as "C direction". If the steel material is a steel pipe, the pipe axis direction is defined as "L direction", the pipe radius direction (wall thickness direction) is defined as "T direction", and the direction that is orthogonal to the L direction and the T direction is defined as "C direction". If the steel material is a round steel bar, the axial direction is defined as "L direction", the radial direction (R direction) is defined as "T direction", and the direction that is orthogonal to the L direction and the T direction is defined as "C direction".

Further, when preparing the test specimen, a test specimen that includes a specified position of the steel material is to be prepared. At such time, the phrase "specified position of the steel material" means a position at which it is possible to stably measure the grain boundary Mo amount γ_{Mo}. Specifically, if the steel material is a steel plate, a thickness t/4 position is defined as the specified position. Note that, in the present description, the term "thickness t/4 position" means the center position between the center portion of the thickness and the surface of the steel plate in the thickness direction. If the steel material is a steel pipe, the center portion of the wall thickness is defined as the specified position. If the steel material is a round steel bar, an R/2 position is defined as the specified position. The size of the test specimen is not particularly limited, and for example the test specimen may have a size that is 10 mm in the L direction × 5 mm in the C direction × 8 mm in the T direction.

The observation surface of the test specimen is mechanically polished, and thereafter is chemically polished with a colloidal silica suspension. On the polished observation surface, a region including the aforementioned specified position is observed using an optical microscope. Specifically, FIG. 3 is a schematic diagram of an observation surface of a test specimen polished in order to determine the grain boundary Mo amount. The L direction and the T direction in FIG. 3 are defined as described above. Referring to FIG. 3, an observation target region 100 of the observation surface of the test specimen after polishing is observed using an optical microscope at a magnification of 200×, and an optical micrograph is obtained. Further, as described above, the observation target region 100 includes the aforementioned specified position. In the observation target region 100, an arbitrary rectangular measurement region 10 of 100 µm × 100 µm is selected. At such time, the measurement region 10 is selected so as to include the aforementioned specified position. Marks 20 are attached at a plurality of corners of the measurement region 10 so that the location of the selected measurement region 10 can be identified. The mark 20 may be, for example, an indentation made by a micro Vickers hardness tester.

Electron backscatter diffraction (EBSD) analysis is performed with respect to the selected measurement region 10 to obtain crystal orientation information with respect to the martensite phase. In the EBSD analysis, the step size is set to 0.1 µm. Grain boundaries (prior-y grain boundaries) of prior-y grains (prior-austenite grains) are identified based on the obtained crystal orientation information and the Kurdjumov-Sachs relationship.

FIG. 4 is a schematic diagram of the measurement region 10 in which prior-y grain boundaries have been identified. Referring to FIG. 4, among the prior-y grain boundaries identified in the measurement region 10, a prior-y grain boundary GB in which the crystal orientation difference between adjacent prior-y grains is 18° or more is selected. A thin film sample TP that is orthogonal to the selected prior-y grain boundary GB is then prepared.

The method for preparing the thin film sample TP will now be described in further detail. FIG. 5 is a schematic diagram illustrating the manner in which the thin film sample TP is prepared from the measurement region 10 illustrated in FIG. 4. As illustrated in FIG. 5, a plate-shaped thin film sample TP having a top face orthogonal to the selected prior-y grain boundary GB is extracted from the measurement region 10 by focused ion beam (FIB) processing. For example, a machine with the trade name "SMI 3050SE" manufactured by Hitachi High-Tech Science Corporation can be used as the FIB processing apparatus.

The extracted thin film sample TP is illustrated in FIG. 6. FIG. 6 is a perspective view of the thin film sample TP illustrated in FIG. 5. In the thin film sample TP, a surface 10 corresponds to one part of the measurement region 10. A surface 30 is a surface which is orthogonal to the surface 10. Naturally, the selected prior-y grain boundary GB at the surface 10 (measurement region 10) is also observed at the surface 30. A thickness T10 of the thin film sample TP is set to 100 nm.

The prepared thin film sample TP is observed using a transmission electron microscope (TEM). In the TEM observation, a TEM equipped with an elemental analyzer (EDS analyzer) that uses energy dispersive X-ray spectrometry (EDS), is used. For example, a transmission electron microscope with a spherical aberration corrector (trade name: NEOARM) manufactured by JEOL Ltd. can be used as the TEM. Further, an EDS analyzer (trade name: JED-2300T) manufactured by JEOL Ltd. can be used as the EDS analyzer attached to the TEM.

FIG. 7 is a schematic diagram for describing the relation between an electron beam and the prior-y grain boundary GB in the thin film sample TP when performing TEM observation and elemental analysis by EDS. As illustrated in FIG. 7, in the TEM observation, first, the thin film sample TP is arranged such that an electron beam EB is incident on the surface 30 of the thin film sample TP. Then, the thin film sample TP is tilted such that the prior-y grain boundary GB of the surface 10 becomes parallel to the incident direction of the electron beam EB. Thereafter, a line segment SL which, as seen from the incident direction of the electron beam EB, has an overall length of 10 nm and which is centered on the prior-y grain boundary GB of the surface 30 and is orthogonal to the prior-y grain boundary GB is specified. Here, one endpoint of the line segment SL is defined as an endpoint E1, and the other endpoint as seen from the incident direction of the electron beam EB is defined as an endpoint E2. The distance between the endpoint E1 and the endpoint E2 will be taken as 10 nm.

Next, elemental analysis by EDS is performed at respective measurement points located at a pitch of 0.2 nm from the endpoint E1 to the endpoint E2 of the line segment SL. The content of Mo (mass%) at each of the measurement points on the line segment SL is determined.

FIG. 8 is a schematic diagram illustrating the relation between the irradiation direction of the electron beam EB when performing TEM observation and elemental analysis by EDS, the prior-y grain boundary GB of the surface 10 of the thin film sample TP, and the element concentration profile. As illustrated in FIG. 8(A), in a case where the electron beam EB is not parallel to the prior-y grain boundary GB of the surface 10 of the thin film sample TP, the peak of an element concentration profile PR on the line segment SL obtained by elemental analysis by EDS is broad. On the other hand, as illustrated in FIG. 8(B), in a case where the electron beam EB is parallel to the prior-y grain boundary GB of the surface 10 of the thin film sample TP, the peak of the element concentration profile PR on the line segment SL is sharp. Therefore, when performing elemental analysis by EDS, the thin film sample TP is tilted such that the electron beam EB becomes parallel to the prior-y grain boundary GB of the surface 10 of the thin film sample TP.

After the content of Mo (mass%) at each measurement point on the line segment SL has been determined by elemental analysis by EDS, the grain boundary Mo amount γ_{Mo} is determined by the following method. FIG. 9 is a view illustrating one example of the content of Mo on the line segment SL which is centered on the prior-y grain boundary GB and which is orthogonal to the prior-y grain boundary GB. Referring to FIG. 9, the respective items shown in FIG. 9 are defined as follows.
- A measurement point at which the content of Mo is maximum on the line segment SL is defined as "Mo peak measurement point P".
- A region having a width of 2.0 nm which is centered on the Mo peak measurement point P is defined as "Mo concentrated region GB0".
- A region between the endpoint E1 of the line segment SL and the Mo concentrated region GB0 is defined as "first Mo intra-grain region BM1".
- A region between the endpoint E2 of the line segment SL and the Mo concentrated region GB0 is defined as "second Mo intra-grain region BM2".
- An arithmetic average value of the contents of Mo at all of the measurement points in the first Mo intra-grain region BM1 is defined as "γ_{Mo1} (mass%)".
- An arithmetic average value of the contents of Mo at all of the measurement points in the second Mo intra-grain region BM2 is defined as "γ_{Mo2} (mass%)".

Referring to FIG. 9, γ_{Mo1} (mass%) in the first Mo intra-grain region BM1 and γ_{Mo2} (mass%) in the second Mo intra-grain region BM2 are regarded as the content of Mo within adjacent prior-y grains that sandwich the prior-y grain boundary GB. In some cases γ_{Mo1} (mass%) and γ_{Mo2} (mass%) will be approximately equal, and in some cases, as in the example in FIG. 9, they will be different concentrations to each other. Therefore, the average of the contents of Mo (γ_{Mo1}, γ_{Mo2}) inside the prior-y grains in each of the first Mo intra-grain region BM1 and the second Mo intra-grain region BM2 is determined.

The grain boundary Mo amount γ_{M0} on the line segment SL is defined by Formula (2) using the content of Mo at each measurement point on the line segment SL, and γ_{Mo1} and γ_{Mo2}. γMo = {(sum total of contents of Mo at all measurement points on line segment SL × 0.2) - γMo1 × (distance between endpoint E1 and Mo peak measurement point P) - γMo2 × (distance between endpoint E2 and Mo peak measurement point P)}/0.8 + (γMo1 + γMo2)/2

Here, Formula (2) is divided as follows. A = (sum total of contents of Mo at all measurement points on line segment SL × 0.2) $B = {γ}_{Mo 1} \times \left(distance between endpoint E1 and Mo peak measurement point P\right)$ $C = {γ}_{Mo 2} \times \left(distance between endpoint E2 and Mo peak measurement point P\right)$ $D = \left({γ}_{Mo 1}+{γ}_{Mo 2}\right) / 2$

The above A corresponds to the total area of the Mo content distribution in FIG. 9, that is, the total amount of the content of Mo on the line segment SL. Note that, in A, "0.2" means 0.2 nm, which is the pitch of the measurement points. B corresponds to the total amount of the content of Mo in a region BM10 that, in the line segment SL, is between the endpoint E1 and the Mo peak measurement point P. γ_{Mo1} (mass%) is used as the average content of Mo in the region BM10. The region BM10 corresponds to an ideal intra-grain region of a prior-y grain in a case where the Mo peak measurement point P is assumed to be an ideal prior-y grain boundary.

C corresponds to the amount of the content of Mo in a region BM20 that, on the line segment SL, is between the endpoint E2 and the Mo peak measurement point P. γ_{Mo2} (mass%) is used as the average content of Mo in the region BM20. The region BM20 corresponds to an ideal intra-grain region of a prior-y grain in a case where the Mo peak measurement point P is assumed to be an ideal prior-y grain boundary. FIG. 10 is a schematic diagram for describing Formula (2). As illustrated in FIG. 10, (A - B - C) among Formula (2) is a value obtained by subtracting the total amount of the contents of Mo in the adjacent ideal intra-grain regions BM10 and BM20 that sandwich the ideal prior-y grain boundary GB from the total amount of the content of Mo on the line segment SL. That is, (A - B - C) in Formula (2) corresponds to a differential amount ΔMo of the content of Mo in the Mo concentrated region GB0 in FIG. 10.

In this connection, as described above, ideally the prior-y grain boundary GB that is orthogonal to the line segment SL does not exist as a wide area (line) like the Mo concentrated region GB0, and instead exists in an extremely narrow area that is centered on the Mo peak measurement point P on the line segment SL. Therefore, in the present description, in the line segment SL, a region with a width of 0.8 nm that is centered on the Mo peak measurement point P is assumed as the region of the prior-y grain boundary GB.

As described above, it is assumed that on the line segment SL, the ideal prior-y grain boundary GB is located in a region with a width of 0.8 nm that is centered on the Mo peak measurement point P, and that as described above, the ideal intra-grain regions BM10 and BM20 are present in regions other than the aforementioned region with a width of 0.8 nm. In this case, it is assumed that the ideal distribution of the content of Mo on the line segment SL is one in which the content of Mo becomes a largest value at the ideal prior-y grain boundary GB, and the content of Mo becomes constant at the average content of Mo in the ideal intra-grain regions BM10 and BM20. The aforementioned D corresponds to the average content of Mo in the ideal intra-grain regions.

Under the assumption described above, a value obtained by adding the average value D of the contents of Mo in the ideal intra-grain regions BM10 and BM20 to a value obtained by dividing ΔMo (= A - B - C) by 0.8, that is, Formula (2), is regarded as the content of Mo (mass%) near the prior-y grain boundary GB. The grain boundary Mo amount γ_{Mo} defined by Formula (2) which is determined by the method described above is an index of the content of Mo near the prior-y grain boundary GB. Note that, a value obtained by rounding off to the first decimal place of the obtained numerical value is adopted as the grain boundary Mo amount (mass%) in the present embodiment.

In the steel material according to the present embodiment, the grain boundary Mo amount defined as described above is 5.0% by mass or more. If the grain boundary Mo amount is too low, the prior-y grain boundaries cannot be strengthened sufficiently, and in a steel material having the chemical composition described above and the yield strength σ_{YS}, the fracture toughness in a low-temperature sour environment cannot be sufficiently increased. On the other hand, if the grain boundary Mo amount is 5.0% by mass or more, on the condition that the other requirements of the present embodiment are satisfied, the fracture toughness in a low-temperature sour environment can be increased.

Therefore, in the present embodiment, on the premise that the steel material has the chemical composition described above and a yield strength σ_{YS} of 758 MPa or more, the grain boundary Mo amount is to be 5.0% by mass or more. A preferable lower limit of the grain boundary Mo amount is 5.5% by mass, more preferably is 6.0% by mass, further preferably is 6.5% by mass, further preferably is 7.0% by mass, further preferably is 7.3% by mass, further preferably is 7.5% by mass, and further preferably is 7.7% by mass. Although the upper limit of the grain boundary Mo amount is not particularly limited, the upper limit of the grain boundary Mo amount may be 30.0% by mass, may be 25.0% by mass, or may be 20.0% by mass.

### [Fn1]

In the steel material according to the present embodiment, in a case where the yield strength σ_{YS} is less than 862 MPa, Fn1 defined by Formula (1) satisfies -300 or more, and in a case where the yield strength σ_{YS} is 862 MPa or more, Fn1 defined by Formula (1) satisfies -520 or more. $Fn 1 = 83 \times \left({γ}_{Mo}-{10}^{- 7}\times √ρ\right) - {σ}_{YS}$

Where, the content of Mo near prior-austenite grain boundaries in percent by mass is substituted for γ_{Mo} in Formula (1), a dislocation density in m⁻² is substituted for ρ in Formula (1), and the yield strength in MPa is substituted for σ_{YS} in Formula (1).

Fn1 (= 83 × (γ_{Mo} - 10⁻⁷ × √ρ) - σ_{YS}) is an index of fracture toughness in a low-temperature sour environment. In a steel material having the chemical composition, the yield strength σ_{YS}, and the grain boundary Mo amount γ_{Mo} which are described above, in a case where the yield strength σ_{YS} is less than 862 MPa, if Fn1 satisfies - 300 or more, the steel material will have excellent fracture toughness even in a low-temperature sour environment. In a steel material having the chemical composition, the yield strength σ_{YS}, and the grain boundary Mo amount γ_{Mo} which are described above, in addition, in a case where the yield strength σ_{YS} is 862 MPa or more, if Fn1 satisfies -520 or more, the steel material will have excellent fracture toughness even in a low-temperature sour environment.

In a case where the yield strength σ_{YS} is less than 862 MPa, a preferable lower limit of Fn1 is -290, more preferably is -280, and further preferably is -270. In a case where the yield strength σ_{YS} is less than 862 MPa, although not particularly limited, the upper limit of Fn1 is, for example, 1606. In a case where the yield strength σ_{YS} is 862 MPa or more, a preferable lower limit of Fn1 is -515, more preferably is -510, further preferably is -505, and further preferably is -500. In a case where the yield strength σ_{YS} is 862 MPa or more, although not particularly limited, the upper limit of Fn1 is, for example, 1408.

Note that, as long as Fn1 satisfies a predetermined value, the dislocation density ρ in Fn1 is not particularly limited. In a steel material having the chemical composition described above, in a case where the yield strength σ_{YS} is less than 862 MPa, the dislocation density ρ is, for example, 2.3×10¹⁴ m⁻² to less than 7.0×10¹⁴ m⁻². In this case, a preferable upper limit of the dislocation density ρ is 6.9×10¹⁴ m⁻², and more preferably is 6.8×10¹⁴ m⁻². In addition, in this case, a preferable lower limit of the dislocation density ρ is more than 2.5×10¹⁴ m⁻², more preferably is more than 2.7×10¹⁴ m⁻², further preferably is 2.8×10¹⁴ m⁻², and further preferably is 3.0×10¹⁴ m⁻². In a steel material having the chemical composition described above, in a case where the yield strength σ_{YS} is 862 MPa or more, the dislocation density ρ is, for example, 7.0×10¹⁴ m⁻² to less than 12.0×10¹⁴ m⁻². In this case, a preferable upper limit of the dislocation density ρ is 11.9×10¹⁴ m⁻², more preferably is 11.5×10¹⁴ m⁻², further preferably is 11.2×10¹⁴ m⁻², and further preferably is 11.0×10¹⁴ m⁻².

The dislocation density ρ of the steel material according to the present embodiment can be determined by the Williamson-Hall method. Specifically, a test specimen for dislocation density measurement is prepared from the steel material according to the present embodiment. If the steel material is a steel plate, the test specimen is prepared from the center portion of the thickness. If the steel material is a steel pipe, the test specimen is prepared from the center portion of the wall thickness. If the steel material is a round steel bar, the test specimen is prepared from an R/2 position. The size of the test specimen is, for example, 20 mm in width × 20 mm in length × 2 mm in thickness. The thickness direction of the test specimen is the thickness direction of the steel material (T direction: thickness direction, pipe radius direction, or radial direction). In this case, the observation surface of the test specimen is a surface with dimensions of 20 mm in width × 20 mm in length. The observation surface of the test specimen is mirror-polished, and furthermore is subjected to electropolishing using a 10 vol% perchloric acid (acetic acid solvent) solution to remove strain from the outer layer. The observation surface after the electropolishing is subjected to X-ray diffraction (XRD) to determine the half-value width ΔK of the peaks of the (110), (211), and (220) planes of the body-centered cubic structure (iron).

In the XRD, measurement of the half-value width ΔK is performed by employing Co Kα radiation as the radiation source, 30 kV as the tube voltage, and 100 mA as the tube current. In addition, LaB₆ (lanthanum hexaboride) powder is used in order to measure a half-value width originating from the X-ray diffractometer.

The heterogeneous strain ε of the test specimen is determined based on the half-value width ΔK determined by the aforementioned method and the Williamson-Hall equation (Formula (3)). $ΔK \times cosθ / λ = 0.9 / D + 2 ε \times sinθ / λ$

Where, in Formula (3), θ represents the diffraction angle, λ represents the wavelength of the X-ray, and D represents the crystallite diameter.

In addition, the dislocation density ρ (m⁻²) can be determined using the obtained heterogeneous strain ε and Formula (4). $ρ = 14.4 \times {ε}^{2} / {b}^{2}$

Where, in Formula (4), b represents the Burgers vector (b = 0.248 (nm)) of the body-centered cubic structure (iron).

### [Fracture toughness in low-temperature sour environment]

The steel material according to the present embodiment has the chemical composition described above, and in the steel material, the yield strength σ_{YS} is 758 MPa or more, the grain boundary Mo amount γ_{Mo} is 5.0% by mass or more, and in a case where the yield strength σ_{YS} is less than 862 MPa, Fn1 satisfies -300 or more, and in a case where the yield strength σ_{YS} is 862 MPa or more, Fn1 satisfies -520 or more. As a result, the steel material according to the present embodiment has a yield strength of 110 ksi or more and has excellent fracture toughness in a low-temperature sour environment. In the present embodiment, excellent fracture toughness in a low-temperature sour environment is evaluated by a DCB test in accordance with NACE TM0177-2016 Method D. Specifically, in the present embodiment, the phrase "has excellent fracture toughness in a low-temperature sour environment" is defined as follows.

A DCB test specimen illustrated in FIG. 11 and a wedge illustrated in FIG. 12 are prepared from the steel material according to the present embodiment. If the steel material is a steel plate, the DCB test specimen and the wedge are prepared from a center portion of the thickness. If the steel material is a steel pipe, the DCB test specimen and the wedge are prepared from a center portion of the wall thickness. If the steel material is a round steel bar, the DCB test specimen and the wedge are prepared from an R/2 position. The longitudinal direction (transverse direction in the drawing) of the DCB test specimen is to be parallel to the L direction (rolling elongation direction, pipe axis direction, or axial direction) of the steel material. A thickness t1 of the wedge is to be 3.10 mm.

Referring to FIG. 11, the prepared wedge is driven in between the arms of the DCB test specimen. The DCB test specimen into which the wedge has been driven is then enclosed in a test vessel. A test solution is poured into the test vessel so as to leave a vapor phase portion, and this is adopted as a test bath. The test solution is a mixed aqueous solution containing 5.0% by mass of sodium chloride and 0.4% by mass of sodium acetate that is adjusted to pH 3.5 using acetic acid (NACE solution B). The amount of the test bath is to be 1 L per test specimen. Next, N₂ gas is blown into the test bath for three hours to degas the test bath until the dissolved oxygen in the test bath becomes 20 ppb or less.

A gaseous mixture consisting of 1% H₂S gas and 99% CO₂ gas is blown as a total pressure of 1 atm into the degassed test bath to make the test bath a corrosive environment. The inside of the test vessel is held at 4°C for 14 days (336 hours) while stirring the test bath. After being held for 14 days, the DCB test specimen is taken out from the test vessel.

A pin is inserted into a hole formed in the tip of the arms of the DCB test specimen that is taken out from the test vessel, a notch portion is opened with a tensile testing machine, and a wedge releasing stress P is measured. In addition, the notch in the DCB test specimen is released in liquid nitrogen, and a crack propagation length "a" of the DCB test specimen with respect to a crack propagation which occurred during immersion in the test bath is measured. The crack propagation length "a" can be measured visually using vernier calipers. A fracture toughness value K_{1SSC} (MPa√m) is determined using Formula (5) based on the measured wedge releasing stress P and the crack propagation length "a". Note that, in Formula (5), h (mm) represents the height of each arm of the DCB test specimen, B (mm) represents the thickness of the DCB test specimen, and Bn (mm) represents the web thickness of the DCB test specimen. These are defined in NACE TM0177-2016 Method D.
FORMULA 1 ${K}_{1 SSC} = \frac{Pa \left(2\sqrt{3}+2.38\frac{h}{a}\right) {\left(\frac{B}{Bn}\right)}^{\frac{1}{\sqrt{3}}}}{{Bh}^{\frac{3}{2}}}$

In the present embodiment, in a case where the yield strength σ_{YS} of the steel material is less than 862 MPa, if the K_{1SSC} value obtained as a result of a DCB test carried out under the conditions described above is 29.5 MPa√m or more, it is determined that the steel material has excellent fracture toughness in a low-temperature sour environment. In addition, in the present embodiment, in a case where the yield strength σ_{YS} of the steel material is 862 MPa or more, if the K_{1SSC} value obtained as a result of a DCB test carried out under the conditions described above is 24.1 MPa√m or more, it is determined that the steel material has excellent fracture toughness in a low-temperature sour environment.

### [Microstructure]

In the microstructure of the steel material according to the present embodiment, the total of the volume ratios of tempered martensite and tempered bainite is 90% or more. The balance of the microstructure is, for example, ferrite or pearlite. If the microstructure of a steel material having the chemical composition described above contains tempered martensite and tempered bainite in an amount equivalent to a total volume ratio of 90% or more, on the condition that the other requirements of the present embodiment are satisfied, the yield strength will be 758 MPa (110 ksi) or more, and the steel material will exhibit excellent fracture toughness in a low-temperature sour environment. That is, in the present embodiment, if the steel material has a yield strength of 758 MPa (110 ksi) or more and has excellent fracture toughness in a low-temperature sour environment, it can be determined that the total of the volume ratios of tempered martensite and tempered bainite in the microstructure is 90% or more.

Note that, the following method can be adopted in the case of determining the volume ratios of tempered martensite and tempered bainite by observation. First, a test specimen having an observation surface is prepared from the steel material according to the present embodiment. If the steel material is a steel plate, a test specimen in which a face including the rolling elongation direction and the thickness direction is adopted as the observation surface is prepared from a center portion of the thickness. If the steel material is a steel pipe, a test specimen in which a face including the pipe axis direction and the pipe radius direction is adopted as the observation surface is prepared from a center portion of the wall thickness. If the steel material is a round steel bar, a test specimen which includes an R/2 position at the center thereof and in which a face including the axial direction and the radial direction is adopted as the observation surface is prepared.

After polishing the observation surface of the test specimen to obtain a mirror surface, the test specimen is immersed for about 10 seconds in a nital etching reagent to reveal the microstructure by etching. The etched observation surface is observed by means of a secondary electron image obtained using a scanning electron microscope (SEM), and observation is performed in 10 visual fields. The area of each visual field is, for example, 0.01 mm² (magnification of 1000×). In each visual field, tempered martensite and tempered bainite are identified based on the contrast. The area fractions of the identified tempered martensite and tempered bainite are determined. The method for determining the area fractions is not particularly limited, and a well-known method can be used. For example, the area fractions of tempered martensite and tempered bainite can be determined by image analysis. In the present embodiment, an arithmetic average value of the area fractions of tempered martensite and tempered bainite determined in all of the visual fields is defined as the volume ratio of tempered martensite and tempered bainite.

### [Shape of steel material]

As described above, the shape of the steel material according to the present embodiment is not particularly limited. The steel material is, for example, a steel pipe, a steel plate, or a round steel bar. In a case where the steel material is an oil-well steel pipe, a preferable wall thickness is 9 to 60 mm. More preferably, the steel material according to the present embodiment is a seamless steel pipe. In a case where the steel material according to the present embodiment is a seamless steel pipe, even when the steel material is a heavy-wall seamless steel pipe with a wall thickness of 15 mm or more, the steel material has a yield strength of 110 ksi or more, and excellent fracture toughness in a low-temperature sour environment.

### [Production method]

A method for producing the steel material according to the present embodiment will now be described. Hereunder, a method for producing a seamless steel pipe as one example of the steel material according to the present embodiment is described. The method for producing a seamless steel pipe includes a process of preparing a hollow shell (preparation process), and a process of subjecting the hollow shell to quenching and tempering to form a seamless steel pipe (quenching process and tempering process). Note that, a production method according to the present embodiment is not limited to the production method described hereunder. Each process is described in detail hereunder.

### [Preparation process]

In the preparation process, an intermediate steel material having the chemical composition described above is prepared. A method for producing the intermediate steel material is not particularly limited as long as the intermediate steel material has the chemical composition described above. As used here, the term "intermediate steel material" refers to a plate-shaped steel material in a case where the end product is a steel plate, refers to a hollow shell in a case where the end product is a steel pipe, and refers to steel material in which a cross section perpendicular to the axial direction is a circular shape in a case where the end product is a round steel bar.

The preparation process may include a process of preparing a starting material (starting material preparation process), and a process of subjecting the starting material to hot working to produce an intermediate steel material (hot working process). Hereunder, a case where the preparation process includes a starting material preparation process and a hot working process is described in detail.

### [Starting material preparation process]

In the starting material preparation process, a starting material is produced using a molten steel having the chemical composition described above. The method for producing the starting material is not particularly limited, and it suffices to use a well-known method. Specifically, a cast piece (a slab, a bloom, or a billet) may be produced by a continuous casting process using the molten steel. An ingot may also be produced by an ingot-making process using the molten steel. As necessary, the slab, bloom, or ingot may be subjected to blooming to produce a billet. A starting material (a slab, a bloom, or a billet) is produced by the above process.

### [Hot working process]

In the hot working process, the prepared starting material is subjected to hot working to produce an intermediate steel material. If the steel material is a seamless steel pipe, the intermediate steel material corresponds to a hollow shell. First, a billet is heated in a heating furnace. Although not particularly limited, the heating temperature is, for example, 1100 to 1300°C. After the billet is extracted from the heating furnace, the billet is subjected to hot working to produce a hollow shell (seamless steel pipe). The method of hot working is not particularly limited, and it suffices to use a well-known method.

For example, the Mannesmann process may be performed as hot working to produce a hollow shell. In this case, a round billet is subjected to piercing-rolling using a piercing machine. When performing piercing-rolling, although not particularly limited, for example, the piercing ratio is 1.0 to 4.0. The round billet subjected to piercing-rolling is further subjected to hot rolling with a mandrel mill, a reducer, a sizing mill, or the like to produce a hollow shell. The cumulative reduction of area in the hot working process is, for example, 20 to 70%.

A hollow shell may be produced from the billet by performing the other hot working methods. For example, in a case where the steel material is a heavy-wall steel material of a short length such as a coupling, a hollow shell may be produced by forging by the Ehrhardt process or the like. A hollow shell is produced by the above process. Although not particularly limited, the wall thickness of the hollow shell is, for example, 9 to 60 mm.

If the steel material is a round steel bar, first, the starting material is heated in a heating furnace. Although not particularly limited, the heating temperature is, for example, 1100 to 1300°C. The starting material extracted from the heating furnace is subjected to hot working to produce an intermediate steel material in which a cross section perpendicular to the axial direction is a circular shape. The hot working is, for example, blooming performed using a blooming mill or hot rolling performed using a continuous mill. In a continuous mill, a horizontal stand having a pair of grooved rolls arranged one on the other in the vertical direction, and a vertical stand having a pair of grooved rolls arranged side by side in the horizontal direction are alternately arranged.

If the steel material is a steel plate, first, the starting material is heated in a heating furnace. Although not particularly limited, the heating temperature is, for example, 1100 to 1300°C. The starting material extracted from the heating furnace is subjected to hot rolling using a blooming mill and a continuous mill to produce an intermediate steel material having a steel plate shape.

The hollow shell produced by hot working may be air-cooled (as-rolled). The hollow shell produced by hot working may be subjected to direct quenching after the hot working without being cooled to normal temperature, or may be subjected to quenching after undergoing supplementary heating (reheating) after the hot working. In a case of performing direct quenching after the hot working, or performing quenching after supplementary heating, cooling may be stopped midway through the quenching process or slow cooling may be performed. In this case, the occurrence of quench cracking in the hollow shell can be suppressed. In addition, in the case of performing direct quenching after hot working, or performing quenching after supplementary heating, stress relief annealing (SR) may be performed at a time that is after quenching and before the heat treatment of the next process. In this case, residual stress of the hollow shell is eliminated.

As described above, an intermediate steel material is prepared in the preparation process. The intermediate steel material may be produced by the aforementioned preferable process, or may be an intermediate steel material produced by a third party, or an intermediate steel material may be prepared that was produced in another factory other than the factory in which a quenching process and a tempering process to be described later are performed or that was produced at different works. Hereunder, the quenching process is described in detail.

### [Quenching process]

In the quenching process, the prepared intermediate steel material (hollow shell) is subjected to quenching. As used in the present description, the term "quenching" means rapidly cooling the intermediate steel material which is at a temperature not lower than the A₃ point. A preferable quenching temperature is 800 to 1000°C. If the quenching temperature is too high, in some cases prior-y grains will become coarse and the SSC resistance of the steel material will decrease. Therefore, a quenching temperature in the range of 800 to 1000°C is preferable.

In the present description, in a case where direct quenching is performed after hot working, the term "quenching temperature" corresponds to the surface temperature of the intermediate steel material that is measured by a thermometer placed on the exit side of the apparatus that performs the final hot working. Further, in a case where quenching is performed after supplementary heating or reheating after hot working, the term "quenching temperature" corresponds to the temperature of the furnace that performs the supplementary heating or reheating.

The quenching method is a method that, for example, continuously cools the intermediate steel material (hollow shell) from the quenching starting temperature and continuously decreases the surface temperature of the hollow shell. The method of performing the continuous cooling treatment is not particularly limited, and a well-known method can be used. The method of performing the continuous cooling treatment is, for example, a method that cools the hollow shell by immersing the hollow shell in a water bath, or a method that cools the hollow shell in an accelerated manner by shower water cooling or mist cooling.

If the cooling rate during quenching is too slow, in some cases the microstructure will not become a microstructure that is principally composed of tempered martensite and tempered bainite. In such a case, the mechanical property defined in the present embodiment (a yield strength of 125 ksi or more) will not be obtained. In such a case, in addition, excellent low-temperature toughness and excellent SSC resistance will not be obtained.

Therefore, as described above, in the method for producing the steel material according to the present embodiment, the intermediate steel material is rapidly cooled during quenching. Specifically, in the quenching process, the average cooling rate when the surface temperature of the intermediate steel material (hollow shell) is within the range of 800 to 500°C during quenching is defined as a "cooling rate during quenching CR₈₀₀₋₅₀₀". More specifically, the cooling rate during quenching CR₈₀₀₋₅₀₀ is determined based on a temperature that is measured at a region that is most slowly cooled within a cross-section of the intermediate steel material that is being quenched (for example, in the case of forcedly cooling both surfaces, the cooling rate is measured at the center portion of the thickness of the intermediate steel material).

A preferable cooling rate during quenching CR₈₀₀₋₅₀₀ is 300°C/min or more. A more preferable lower limit of the cooling rate during quenching CR₈₀₀₋₅₀₀ is 450°C/min, and further preferably is 600°C/min. Although an upper limit of the cooling rate during quenching CR₈₀₀₋₅₀₀ is not particularly defined, the upper limit is, for example, 60000°C/min.

Preferably, quenching is performed after performing heating of the hollow shell in the austenite zone a plurality of times. In this case, the SSC resistance of the steel material increases because austenite grains are refined prior to quenching. Heating in the austenite zone may be repeated a plurality of times by performing quenching a plurality of times, or heating in the austenite zone may be repeated a plurality of times by performing normalizing and quenching. Further, quenching and tempering to be described later may be performed in combination a plurality of times. That is, both quenching and tempering may be performed a plurality of times. In such a case, the SSC resistance of the steel material increases further. The tempering process is described in detail hereunder.

### [Tempering process]

The tempering process is carried out by performing tempering after performing the aforementioned quenching. In the present description, the term "tempering" means reheating the intermediate steel material after quenching to a temperature that is less than the A_{c1} point and holding the intermediate steel material at that temperature. Here, the term "holding temperature" corresponds to the temperature of the furnace when the intermediate steel material after quenching is heated and held at the relevant temperature. The term "holding time" means the period of time from the temperature of the intermediate steel material reaching a predetermined holding temperature until the steel material is extracted from the heat treatment furnace.

In the case of producing a steel material that is to be used for oil wells, conventionally the holding temperature has been set within a range of 630 to 730°C for the purpose of increasing the SSC resistance and the like. On the other hand, as a result of detailed studies by the present inventors, it was revealed that Mo can be selectively concentrated at prior-y grain boundaries by performing tempering at a temperature within a range of 450 to 600°C, which is lower than the temperature at which tempering is generally performed. Therefore, in the tempering process according to the present embodiment, tempering is performed in the range of 450 to 600°C. On the other hand, when tempering is merely performed at a temperature in the range of 450 to 600°C, in some cases the dislocation density ρ becomes too high and Fn1 decreases too much.

Therefore, in the tempering process according to the present embodiment, tempering at a temperature in the range of 450 to 600°C is performed for a holding time of a certain extent or more and the diffusion length with respect to the overall tempering is increased. Specifically, in the present embodiment, a diffusion length √Dt during tempering is defined by the following Formula (6).
FORMULA 2 $\sqrt{Dt} = \sqrt{0.0002 \times exp \left(\frac{- 240900 \times \left(1+0.222\times {s}^{2}\right)}{8.314 \times \left(273.15+T\right)}\right) \times t}$

In addition, s² in Formula (6) is defined by the following Formula (7).
FORMULA 3 $\begin{matrix}{s}^{2} = - 1.20745921 \times {10}^{- 10} \times {\left(T+273.15\right)}^{4} \\ + 4.13480963 \times {10}^{- 7} \times {\left(T+273.15\right)}^{3} \\ - 5.33104487 \times {10}^{- 4} \times {\left(T+273.15\right)}^{2} \\ + 0.305049675 \times \left(T+273.15\right) - 64.4602206\end{matrix}$

Note that, the holding temperature during tempering is substituted in °C for T in Formulae (6) and (7), and the holding time during tempering is substituted in seconds for t in Formula (6).

More specifically, in the present embodiment, a diffusion length during tempering in the range of 450 to 600°C is defined as "diffusion length √Dt_{L}". In the present embodiment, preferably the diffusion length √Dt_{L} during tempering in the range of 450 to 600°C is 1.3 nm or more, and a diffusion length √Dt_{To} in the overall tempering is 60.0 nm or more. The process for performing tempering is not particularly limited as long as the diffusion lengths √Dt_{L} and √Dt_{To} satisfy the aforementioned ranges. For example, so-called "tempering in two stages" in which tempering is first performed at a high temperature and thereafter tempering is performed at a temperature in the range of 450 to 600°C may be performed. Further, for example, only tempering at a temperature in the range of 450 to 600°C may be performed.

Hereunder, each process in a case where tempering at a high temperature (high-temperature tempering process) is performed and thereafter tempering at a temperature in the range of 450 to 600°C (hereunder, also referred to as "intermediate-temperature tempering") is performed is described separately.

### [High-temperature tempering process]

In the case of performing a high-temperature tempering process, the intermediate steel material (hollow shell) subjected to quenching is heated from room temperature to the holding temperature, and thereafter is held at the holding temperature for the holding time. In the high-temperature tempering process, a preferable holding temperature is 640 to 740°C. A more preferable lower limit of the holding temperature in the high-temperature tempering process is 645°C, and further preferably is 650°C. A more preferable upper limit of the holding temperature in the high-temperature tempering process is 730°C. In the high-temperature tempering process according to the present embodiment, a preferable holding time is 5 to 120 minutes. A more preferable upper limit of the holding time in the high-temperature tempering process is 100 minutes. A more preferable lower limit of the holding time in the high-temperature tempering process is 10 minutes, and further preferably is 20 minutes.

In the present embodiment, in the case of performing the high-temperature tempering process, a diffusion length in the high-temperature tempering process is defined as "√Dt_{H}". Here, √Dt_{H} can be determined using the holding temperature (°C) and holding time (seconds) in the high-temperature tempering process, and the aforementioned Formulae (6) and (7). In the present embodiment, the diffusion length √Dt_{H} in the high-temperature tempering process is not particularly limited.

### [Intermediate-temperature tempering process]

In the intermediate-temperature tempering process, the intermediate steel material (hollow shell) is held at 450 to 600°C. In the intermediate-temperature tempering process, holding the intermediate steel material (hollow shell) at 450 to 600°C causes Mo to concentrate at prior-y grain boundaries. At such time, a preferable holding time is 100 minutes or more. If the holding time in the intermediate-temperature tempering process is too short, in some cases the grain boundary Mo amount will not be sufficiently increased in the produced steel material. Although not particularly limited, an upper limit of the holding time may be, for example, 8,333 hours.

In the intermediate-temperature tempering process according to the present embodiment, it is preferable to make the diffusion length √Dt_{L} a length of 1.3 nm or more. If the diffusion length √Dt_{L} is too small, in some cases the grain boundary Mo amount will not be sufficiently increased in the produced steel material. Therefore, in the intermediate-temperature tempering process according to the present embodiment, a preferable lower limit of the diffusion length √Dt_{L} is 1.3 nm or more. Note that, although not particularly limited, an upper limit of the diffusion length √Dt_{L} is, for example, 250.0 nm.

In the case of performing tempering in two stages, the diffusion length √Dt_{To} in the overall tempering can be determined as the square root of sum of squares of the diffusion length √Dt_{H} in the high-temperature tempering process and the diffusion length √Dt_{L} in the intermediate-temperature tempering process. Specifically, the diffusion length √Dt_{To} can be determined using the following Formula (8).
FORMULA 4 $\sqrt{{Dt}_{To}} = \sqrt{{\sqrt{{Dt}_{H}}}^{2} + {\sqrt{{Dt}_{L}}}^{2}}$

Note that, as described above, the tempering process according to the present embodiment may be carried out by performing only the intermediate-temperature tempering process. In such a case, the diffusion length √Dt_{To} in the overall tempering is the same as the diffusion length √Dt_{L} in the intermediate-temperature tempering process. Further, the tempering process according to the present embodiment may be carried out by performing tempering in three stages or more. Even in such a case, it is preferable to make the diffusion length √Dt_{L} in the intermediate-temperature tempering process 1.3 nm or more, and to make the diffusion length √Dt_{To} in overall tempering 60.0 nm or more.

Further, in the tempering process, the holding temperature and holding time are appropriately adjusted to obtain a steel material having a yield strength of 758 MPa or more. Here, those skilled in the art are fully capable of subjecting an intermediate steel material (hollow shell) having the chemical composition of the present embodiment to tempering in which the aforementioned holding temperature and aforementioned holding time have been appropriately adjusted to make the yield strength 758 MPa or more.

The steel material according to the present embodiment can be produced according to the production method described above. In the foregoing description of the production method, a method for producing a seamless steel pipe as one example of the steel material according to the present embodiment has been described. However, the steel material according to the present embodiment may also be a steel plate or in another shape. A method for producing a steel plate or a steel material in another shape also includes, for example, a preparation process, a quenching process, and a tempering process, similarly to the production method described above. However, the production method described above is an example, and the steel material according to the present embodiment may also be produced by the other production methods. Hereunder, the present disclosure is described more specifically by way of examples.

### EXAMPLE 1

In Example 1, steel materials having a yield strength of less than 862 MPa were investigated. Specifically, molten steels which each had a weight of 180 kg and had the chemical compositions shown in Table 1-1 and Table 1-2 were produced. Note that, the symbol "-" in Table 1-2 means that contents of the respective elements are at the level of an impurity. Specifically, "-" means that the content of Co, the content of W, the content of Ni, and the content of Cu of Test No. 1-1 were each 0% when rounded off to second decimal place. In addition, "-" means that the content of Nb of Test No. 1-1 was 0% when rounded off to third decimal place. Further, "-" means that the content of Ca, the content of Mg, the content of Zr, and the content of REM of Test No. 1-1 were each 0% when rounded off to fourth decimal place.

### [Table 1-1]

**TABLE 1-1**

| Test Number | Chemical Composition (unit is mass%; balance is Fe and impurities) | | | | | | | | | | |
|---|---|---|---|---|---|---|---|---|---|---|---|
| | C | Si | Mn | P | S | Al | Cr | Mo | V | Ti | B |
| 1-1 | 0.29 | 0.71 | 0.14 | 0.006 | 0.0007 | 0.025 | 0.95 | 0.81 | 0.16 | 0.010 | 0.0015 |
| 1-2 | 0.40 | 1.07 | 0.06 | 0.008 | 0.0010 | 0.036 | 0.72 | 1.05 | 0.16 | 0.010 | 0.0014 |
| 1-3 | 0.25 | 0.24 | 0.06 | 0.009 | 0.0009 | 0.045 | 0.93 | 1.00 | 0.08 | 0.009 | 0.0015 |
| 1-4 | 0.26 | 0.99 | 0.27 | 0.009 | 0.0008 | 0.054 | 1.24 | 0.51 | 0.20 | 0.010 | 0.0013 |
| 1-5 | 0.31 | 1.39 | 0.24 | 0.011 | 0.0010 | 0.041 | 0.47 | 1.23 | 0.06 | 0.018 | 0.0011 |
| 1-6 | 0.26 | 1.20 | 0.28 | 0.007 | 0.0010 | 0.031 | 0.71 | 0.98 | 0.11 | 0.014 | 0.0011 |
| 1-7 | 0.25 | 1.35 | 0.30 | 0.009 | 0.0009 | 0.048 | 0.67 | 0.82 | 0.14 | 0.010 | 0.0012 |
| 1-8 | 0.35 | 0.42 | 0.42 | 0.008 | 0.0007 | 0.035 | 0.86 | 1.07 | 0.08 | 0.013 | 0.0014 |
| 1-9 | 0.37 | 0.83 | 0.16 | 0.012 | 0.0010 | 0.032 | 0.89 | 0.67 | 0.15 | 0.009 | 0.0013 |
| 1-10 | 0.35 | 1.01 | 0.43 | 0.007 | 0.0006 | 0.029 | 0.67 | 1.03 | 0.16 | 0.011 | 0.0015 |
| 1-11 | 0.46 | 0.54 | 0.29 | 0.010 | 0.0008 | 0.055 | 0.80 | 0.62 | 0.11 | 0.009 | 0.0013 |
| 1-12 | 0.45 | 1.09 | 0.12 | 0.007 | 0.0009 | 0.036 | 1.05 | 0.55 | 0.09 | 0.012 | 0.0011 |
| 1-13 | 0.39 | 1.31 | 0.35 | 0.010 | 0.0008 | 0.042 | 0.90 | 0.58 | 0.08 | 0.013 | 0.0014 |
| 1-14 | 0.49 | 0.22 | 0.10 | 0.006 | 0.0006 | 0.040 | 1.01 | 0.94 | 0.09 | 0.010 | 0.0014 |
| 1-15 | 0.27 | 1.35 | 0.41 | 0.010 | 0.0008 | 0.035 | 0.98 | 0.67 | 0.11 | 0.011 | 0.0012 |
| 1-16 | 0.26 | 1.09 | 0.42 | 0.011 | 0.0006 | 0.052 | 0.91 | 0.59 | 0.09 | 0.010 | 0.0012 |
| 1-17 | 0.35 | 1.37 | 0.34 | 0.011 | 0.0008 | 0.049 | 0.98 | 0.75 | 0.10 | 0.011 | 0.0014 |
| 1-18 | 0.31 | 0.50 | 0.31 | 0.010 | 0.0009 | 0.032 | 1.09 | 1.35 | 0.08 | 0.013 | 0.0015 |
| 1-19 | 0.25 | 0.77 | 0.43 | 0.006 | 0.0010 | 0.055 | 1.14 | 1.17 | 0.15 | 0.009 | 0.0013 |
| 1-20 | 0.27 | 1.19 | 0.44 | 0.012 | 0.0006 | 0.047 | 0.85 | 0.67 | 0.10 | 0.012 | 0.0015 |
| 1-21 | 0.25 | 1.17 | 0.32 | 0.011 | 0.0007 | 0.050 | 0.88 | 0.56 | 0.13 | 0.012 | 0.0014 |
| 1-22 | 0.32 | 0.40 | 0.17 | 0.006 | 0.0007 | 0.055 | 0.01 | 0.50 | 0.16 | 0.010 | 0.0015 |
| 1-23 | 0.40 | 0.64 | 0.23 | 0.008 | 0.0009 | 0.025 | 0.53 | 0.02 | 0.16 | 0.012 | 0.0011 |
| 1-24 | 0.35 | 1.16 | 0.97 | 0.012 | 0.0010 | 0.039 | 0.95 | 0.82 | 0.10 | 0.013 | 0.0014 |
| 1-25 | 0.41 | 1.16 | 0.09 | 0.011 | 0.0008 | 0.055 | 0.53 | 0.95 | 0.14 | 0.014 | 0.0012 |
| 1-26 | 0.30 | 0.41 | 0.25 | 0.066 | 0.0010 | 0.042 | 0.56 | 0.87 | 0.16 | 0.015 | 0.0014 |

### [Table 1-2]

**TABLE 1-2**

| Test Number | Chemical Composition (unit is mass%; balance is Fe and impurities) | | | | | | | | | | |
|---|---|---|---|---|---|---|---|---|---|---|---|
| | N | O | Nb | Ca | Mg | Zr | REM | Co | W | Ni | Cu |
| 1-1 | 0.0032 | 0.0006 | - | - | - | - | - | - | - | - | - |
| 1-2 | 0.0025 | 0.0017 | - | - | - | - | - | - | - | - | - |
| 1-3 | 0.0026 | 0.0018 | - | - | - | - | - | - | - | - | - |
| 1-4 | 0.0046 | 0.0018 | - | - | - | - | - | - | - | - | - |
| 1-5 | 0.0029 | 0.0009 | - | - | - | - | - | - | - | - | - |
| 1-6 | 0.0032 | 0.0018 | 0.016 | - | - | - | - | - | - | - | - |
| 1-7 | 0.0026 | 0.0012 | - | 0.0019 | - | - | - | - | - | - | - |
| 1-8 | 0.0037 | 0.0009 | - | - | 0.0017 | - | - | - | - | - | - |
| 1-9 | 0.0023 | 0.0007 | - | - | - | 0.0014 | - | - | - | - | - |
| 1-10 | 0.0036 | 0.0015 | - | - | - | - | 0.0021 | - | - | - | - |
| 1-11 | 0.0047 | 0.0009 | - | - | - | - | - | 0.26 | - | - | - |
| 1-12 | 0.0028 | 0.0007 | - | - | - | - | - | - | 0.24 | - | - |
| 1-13 | 0.0024 | 0.0011 | - | - | - | - | - | - | - | 0.05 | - |
| 1-14 | 0.0026 | 0.0016 | - | - | - | - | - | - | - | - | 0.24 |
| 1-15 | 0.0040 | 0.0016 | - | - | - | - | - | - | - | - | - |
| 1-16 | 0.0031 | 0.0006 | 0.011 | - | - | - | - | - | - | - | - |
| 1-17 | 0.0022 | 0.0012 | - | - | - | - | - | - | - | - | - |
| 1-18 | 0.0032 | 0.0007 | - | - | - | - | - | - | - | - | - |
| 1-19 | 0.0035 | 0.0007 | - | - | - | - | - | - | - | - | - |
| 1-20 | 0.0044 | 0.0009 | - | - | - | - | - | - | - | - | - |
| 1-21 | 0.0031 | 0.0017 | - | - | - | - | - | - | - | - | - |
| 1-22 | 0.0037 | 0.0007 | - | - | - | - | - | - | - | - | - |
| 1-23 | 0.0047 | 0.0015 | - | - | - | - | - | - | - | - | - |
| 1-24 | 0.0031 | 0.0006 | - | - | - | - | - | - | - | - | - |
| 1-25 | 0.0510 | 0.0007 | - | - | - | - | - | - | - | - | - |
| 1-26 | 0.0024 | 0.0015 | - | - | - | - | - | - | - | - | - |

Ingots were produced using the molten steels of Test Nos. 1-1 to 1-26. The produced ingots were subjected to hot rolling to produce steel plates having a thickness of 15 mm. The steel plates of Test Nos. 1-1 to 1-26 after hot rolling were allowed to cool to bring the temperature of the steel plate to normal temperature (25°C). After being allowed to cool, the steel plates of Test Nos. 1-1 to 1-26 were held for 20 minutes at the quenching temperature (920°C), and thereafter the steel plates were immersed in a water bath to be quenched. At this time, the cooling rate during quenching (CR₈₀₀₋₅₀₀) was 600°C/min for each test number. Note that, a type K thermocouple of a sheath type was inserted into a center portion of the thickness of the steel plate in advance, and the quenching temperature and cooling rate during quenching CR₈₀₀₋₅₀₀ were measured using the type K thermocouple.

After quenching, the steel plates of Test Nos. 1-1 to 1-26 were subjected to tempering. In the present example, tempering at a high temperature is also referred to as "first tempering", and tempering at an intermediate temperature is also referred to as "second tempering". The holding temperature (°C), holding time (minutes), and diffusion length (√Dt_{H} (nm) or √Dt_{L} (nm)) for the first tempering and the second tempering are shown in Table 2. In addition, the diffusion length √Dt_{To} (nm) in the overall tempering as determined based on the diffusion lengths √Dt_{H} and √Dt_{L} and Formula (8) is shown in Table 2. Note that, in Table 2, the symbol "-" in the column "First Tempering" means that the first tempering was not performed. Similarly, in Table 2, the symbol "-" in the column "Second Tempering" means that the second tempering was not performed.

### [Table 2]

**TABLE 2**

| Test Number | First Tempering | | | Second Tempering | | | Overall Tempering √D_{To} (nm) |
|---|---|---|---|---|---|---|---|
| | Holding Temperature (°C) | Holding Time (min) | √Dt_{H} (nm) | Holding Temperature (°C) | Holding Time (min) | √Dt_{L} (nm) | |
| 1-1 | 720 | 60 | 177.6 | 550 | 900 | 7.0 | 177.7 |
| 1-2 | 720 | 60 | 177.6 | 550 | 900 | 7.0 | 177.7 |
| 1-3 | - | - | - | 550 | 129600 | 84.4 | 84.4 |
| 1-4 | 720 | 60 | 177.6 | 550 | 900 | 7.0 | 177.7 |
| 1-5 | 720 | 60 | 177.6 | 550 | 900 | 7.0 | 177.7 |
| 1-6 | 720 | 60 | 177.6 | 550 | 900 | 7.0 | 177.7 |
| 1-7 | 710 | 40 | 111.2 | 550 | 900 | 7.0 | 111.4 |
| 1-8 | 720 | 40 | 145.0 | 600 | 180 | 13.3 | 145.6 |
| 1-9 | 720 | 60 | 177.6 | 550 | 600 | 5.7 | 177.7 |
| 1-10 | 720 | 80 | 205.1 | 550 | 900 | 7.0 | 205.2 |
| 1-11 | 720 | 70 | 191.8 | 550 | 900 | 7.0 | 191.9 |
| 1-12 | 720 | 80 | 205.1 | 550 | 900 | 7.0 | 205.2 |
| 1-13 | 720 | 90 | 217.5 | 550 | 500 | 5.2 | 217.6 |
| 1-14 | 720 | 90 | 217.5 | 500 | 2880 | 2.6 | 217.5 |
| 1-15 | 720 | 90 | 217.5 | - | - | - | 217.5 |
| 1-16 | 710 | 80 | 157.3 | - | - | - | 157.3 |
| 1-17 | 720 | 90 | 217.5 | 680 | 30 | 44.3 | 222.0 |
| 1-18 | 710 | 60 | 136.2 | 570 | 40 | 2.7 | 136.2 |
| 1-19 | 710 | 60 | 136.2 | 560 | 80 | 2.8 | 136.2 |
| 1-20 | 700 | 60 | 104.9 | 500 | 80 | 0.4 | 104.9 |
| 1-21 | 700 | 60 | 104.9 | 500 | 180 | 0.7 | 104.9 |
| 1-22 | 720 | 60 | 177.6 | 550 | 900 | 7.0 | 177.7 |
| 1-23 | 710 | 60 | 136.2 | 550 | 900 | 7.0 | 136.4 |
| 1-24 | 720 | 80 | 205.1 | 550 | 900 | 7.0 | 205.2 |
| 1-25 | 720 | 80 | 205.1 | 550 | 900 | 7.0 | 205.2 |
| 1-26 | 720 | 60 | 177.6 | 550 | 900 | 7.0 | 177.7 |

Here, the temperature of the heat treatment furnace where tempering was performed was adopted as the holding temperature during tempering in the present example. In addition, the holding time during tempering in the present example was taken as the time from when the temperature of the steel plate of each test number reached a predetermined tempering temperature until the steel plate was extracted from the heat treatment furnace.

### [Evaluation tests]

The steel plates of Test Nos. 1-1 to 1-26 on which tempering had been performed were subjected to a tensile test, a dislocation density measurement test, a grain boundary Mo amount measurement test, and a DCB test that are described hereunder.

### [Tensile test]

The steel plates of Test Nos. 1-1 to 1-26 were subjected to a tensile test by the method described above. Specifically, a round bar tensile test specimen having a parallel portion diameter of 4 mm and a gage length of 16 mm was prepared from a center portion of the thickness of each steel plate of Test Nos. 1-1 to 1-26. The axial direction of the round bar tensile test specimen was parallel to the rolling elongation direction of the steel plate. Using the round bar specimens of Test Nos. 1-1 to 1-26, a tensile test in accordance with ASTM E8/E8M (2021) was carried out at normal temperature (25°C) in the atmosphere, and the yield strength (MPa) of each steel plate of Test Nos. 1-1 to 1-26 was determined. The obtained yield strength is shown as "Yield Strength σ_{YS} (MPa)" in Table 3.

### [Table 3]

**TABLE 3**

| Test Number | Yield Strength σ_{YS} (MPa) | Dislocation Density ρ (10¹⁴ m⁻²) | Grain Boundary Mo Amount γ_{Mo} (mass%) | Fn1 | K_{1SSC} (MPa√m) |
|---|---|---|---|---|---|
| 1-1 | 794 | 4.2 | 10.5 | -93 | 34.1 |
| 1-2 | 835 | 4.2 | 10.8 | -109 | 32.9 |
| 1-3 | 816 | 5.8 | 19.7 | 619 | 38.2 |
| 1-4 | 805 | 4.6 | 8.6 | -269 | 30.7 |
| 1-5 | 821 | 4.9 | 10.9 | -100 | 33.1 |
| 1-6 | 804 | 4.8 | 9.1 | -231 | 32.8 |
| 1-7 | 854 | 6.8 | 10.5 | -199 | 32.7 |
| 1-8 | 792 | 3.5 | 15.3 | 323 | 37.5 |
| 1-9 | 814 | 4.0 | 8.9 | -241 | 30.8 |
| 1-10 | 785 | 3.2 | 10.3 | -79 | 33.8 |
| 1-11 | 816 | 3.0 | 9.4 | -180 | 34.0 |
| 1-12 | 816 | 3.1 | 10.0 | -132 | 33.6 |
| 1-13 | 801 | 3.3 | 8.3 | -263 | 32.3 |
| 1-14 | 806 | 2.4 | 8.1 | -262 | 31.0 |
| 1-15 | 761 | 7.2 | 5.4 | -536 | 28.2 |
| 1-16 | 806 | 8.8 | 5.1 | -629 | 28.1 |
| 1-17 | 789 | 7.5 | 5.9 | -527 | 27.0 |
| 1-18 | 814 | 8.4 | 8.2 | -374 | 28.2 |
| 1-19 | 798 | 7.7 | 8.3 | -339 | 28.3 |
| 1-20 | 849 | 9.3 | 5.3 | -662 | 26.4 |
| 1-21 | 841 | 6.7 | 5.5 | -599 | 26.6 |
| 1-22 | 775 | 3.2 | 9.7 | -118 | 19.4 |
| 1-23 | 806 | 3.2 | 0.3 | -930 | 16.9 |
| 1-24 | 786 | 3.2 | 8.9 | -196 | 14.6 |
| 1-25 | 810 | 3.4 | 9.6 | -166 | 20.3 |
| 1-26 | 774 | 3.3 | 9.2 | -161 | 12.4 |

### [Dislocation density measurement test]

The steel plates of Test Nos. 1-1 to 1-26 were subjected to a dislocation density measurement test by the method described above. Specifically, a test specimen having dimensions of 20 mm in width × 20 mm in length × 2 mm in thickness was prepared from a center portion of the thickness of each steel plate of Test Nos. 1-1 to 1-26. The half-value width ΔK of the peaks of the (110), (211), and (220) planes was determined using X-ray diffraction according to the method described above. The determined half-value widths ΔK were used to determine the dislocation density ρ (m⁻²) by the method described above. The obtained dislocation density is shown as "Dislocation Density ρ (10¹⁴ m⁻²)" in Table 3.

### [Grain boundary Mo amount measurement test]

The steel plates of Test Nos. 1-1 to 1-26 were subjected to a grain boundary Mo amount measurement test by the method described above. Specifically, for each of the steel plates of Test Nos. 1-1 to 1-26, a test specimen was prepared which included a thickness t/4 position at the center thereof and which had a size having a length of 10 mm in the rolling elongation direction × 5 mm in the width direction × 8 mm in the thickness direction. The prepared test specimen was used to determine the grain boundary Mo amount (mass%) by the method described above. The obtained grain boundary Mo amount is shown as "Grain Boundary Mo Amount γ_{Mo} (mass%)" in Table 3. In addition, Fnl was obtained using the obtained yield strength σ_{YS} (MPa), dislocation density ρ (m⁻²), and grain boundary Mo amount γ_{Mo} (mass%), and Formula (1). The obtained Fn1 is shown in Table 3.

### [DCB test]

The steel plates of Test Nos. 1-1 to 1-26 were subjected to a DCB test by the method described above. Specifically, a DCB test specimen and a wedge that are described above were prepared from a center portion of the thickness of each of the steel plates of Test Nos. 1-1 to 1-26. A DCB test in accordance with NACE TM0177-2016 Method D was performed under the conditions described above using the prepared test specimen and wedge. The fracture toughness value K_{1SSC} obtained by the DCB test carried out according to the method described above is shown as "K_{1SSC} (MPa√m)" in Table 3.

### [Evaluation results]

Referring to Table 1-1, Table 1-2, Table 2, and Table 3, in each of the steel plates of Test Nos. 1-1 to 1-14, the chemical composition was appropriate and the yield strength was 758 MPa or more (110 ksi or more). In addition, the grain boundary Mo amount γ_{Mo} was 5.0% by mass or more and Fnl was -300 or more. As a result, the K_{1SSC} value was 29.5 MPa or more. That is, these steel plates had a yield strength of 110 ksi or more, and had excellent fracture toughness in a low-temperature sour environment.

On the other hand, the steel plates of Test Nos. 1-15 and 1-16 were not subjected to an intermediate-temperature tempering process. As a result, for these steel plates, Fnl was less than -300. Consequently, the K_{1SSC} value of each of these steel plates was less than 29.5 MPa. That is, these steel plates did not have excellent fracture toughness in a low-temperature sour environment.

For the steel plate of Test No. 1-17, in the intermediate-temperature tempering process, the holding temperature was too high and the holding time was too short. As a result, for this steel plate, Fnl was less than -300. Consequently, the K_{1SSC} value of this steel plate was less than 29.5 MPa. That is, this steel plate did not have excellent fracture toughness in a low-temperature sour environment.

For the steel plates of Test Nos. 1-18 and 1-19, the holding time in the intermediate-temperature tempering process was too short. As a result, for these steel plates, Fnl was less than -300. Consequently, the K_{1SSC} value for each of these steel plates was less than 29.5 MPa. That is, these steel plates did not have excellent fracture toughness in a low-temperature sour environment.

For the steel plate of Test No. 1-20, in the intermediate-temperature tempering process, the holding time was too short and the diffusion length √Dt_{L} was too small. As a result, for this steel plate, Fn1 was less than -300. Consequently, the K_{1SSC} value of this steel plate was less than 29.5 MPa. That is, this steel plate did not have excellent fracture toughness in a low-temperature sour environment.

For the steel plate of Test No. 1-21, the diffusion length √Dt_{L} in the intermediate-temperature tempering process was too small. As a result, for this steel plate, Fnl was less than -300. Consequently, the K_{1SSC} value of this steel plate was less than 29.5 MPa. That is, this steel plate did not have excellent fracture toughness in a low-temperature sour environment.

In the steel plate of Test No. 1-22, the content of Cr was too low. As a result, the K_{1SSC} value of this steel plate was less than 29.5 MPa. That is, this steel plate did not have excellent fracture toughness in a low-temperature sour environment.

In the steel plate of Test No. 1-23, the content of Mo was too low. As a result, in this steel plate, the grain boundary Mo amount mₑ was less than 5.0% by mass, and Fnl was less than -300. Consequently, the K_{1SSC} value of this steel plate was less than 29.5 MPa. That is, this steel plate did not have excellent fracture toughness in a low-temperature sour environment.

In the steel plate of Test No. 1-24, the content of Mn was too high. As a result, the K_{1SSC} value of this steel plate was less than 29.5 MPa. That is, this steel plate did not have excellent fracture toughness in a low-temperature sour environment.

In the steel plate of Test No. 1-25, the content of N was too high. As a result, the K_{1SSC} value of this steel plate was less than 29.5 MPa. That is, this steel plate did not have excellent fracture toughness in a low-temperature sour environment.

In the steel plate of Test No. 1-26, the content of P was too high. As a result, the K_{1SSC} value of this steel plate was less than 29.5 MPa. That is, this steel plate did not have excellent fracture toughness in a low-temperature sour environment.

### EXAMPLE 2

In Example 2, steel materials having a yield strength of 862 MPa or more were investigated. Specifically, molten steels having a weight of 180 kg and the chemical compositions shown in Table 4-1 and Table 4-2 were produced. Note that, the symbol "-" in Table 4-2 means that the contents of the respective elements are at the level of an impurity. Specifically, "-" means that the content of Co, the content of W, the content of Ni, and the content of Cu of Test No. 2-1 were each 0% when rounded off to second decimal place. In addition, "-" means that the content of Nb of Test No. 2-1 was 0% when rounded off to third decimal place. Further, "-" means that the content of Ca, the content of Mg, the content of Zr, and the content of REM of Test No. 2-1 were each 0% when rounded off to fourth decimal place.

### [Table 4-1]

**TABLE 4-1**

| Test Number | Chemical Composition (unit is mass%; balance is Fe and impurities) | | | | | | | | | | |
|---|---|---|---|---|---|---|---|---|---|---|---|
| | C | Si | Mn | P | S | Al | Cr | Mo | V | Ti | B |
| 2-1 | 0.28 | 1.09 | 0.18 | 0.009 | 0.0006 | 0.032 | 0.77 | 0.91 | 0.11 | 0.011 | 0.0014 |
| 2-2 | 0.45 | 1.17 | 0.13 | 0.008 | 0.0009 | 0.041 | 0.54 | 0.75 | 0.16 | 0.015 | 0.0012 |
| 2-3 | 0.29 | 1.14 | 0.06 | 0.012 | 0.0008 | 0.029 | 0.62 | 1.04 | 0.12 | 0.013 | 0.0013 |
| 2-4 | 0.25 | 1.37 | 0.14 | 0.006 | 0.0010 | 0.030 | 1.22 | 0.52 | 0.19 | 0.018 | 0.0011 |
| 2-5 | 0.32 | 0.98 | 0.41 | 0.007 | 0.0007 | 0.051 | 0.44 | 1.25 | 0.07 | 0.010 | 0.0011 |
| 2-6 | 0.40 | 0.33 | 0.33 | 0.007 | 0.0009 | 0.028 | 0.86 | 1.18 | 0.09 | 0.009 | 0.0012 |
| 2-7 | 0.37 | 1.28 | 0.40 | 0.010 | 0.0008 | 0.055 | 0.64 | 0.74 | 0.10 | 0.010 | 0.0012 |
| 2-8 | 0.34 | 1.09 | 0.42 | 0.007 | 0.0010 | 0.032 | 0.65 | 0.58 | 0.12 | 0.013 | 0.0014 |
| 2-9 | 0.33 | 0.79 | 0.33 | 0.007 | 0.0006 | 0.043 | 0.81 | 0.93 | 0.12 | 0.013 | 0.0013 |
| 2-10 | 0.32 | 1.29 | 0.25 | 0.007 | 0.0009 | 0.035 | 1.03 | 0.67 | 0.12 | 0.009 | 0.0011 |
| 2-11 | 0.31 | 0.99 | 0.27 | 0.008 | 0.0007 | 0.036 | 0.60 | 1.02 | 0.10 | 0.009 | 0.0013 |
| 2-12 | 0.29 | 0.83 | 0.06 | 0.012 | 0.0006 | 0.025 | 0.73 | 0.69 | 0.10 | 0.010 | 0.0011 |
| 2-13 | 0.43 | 0.41 | 0.25 | 0.008 | 0.0009 | 0.029 | 0.93 | 0.54 | 0.16 | 0.014 | 0.0011 |
| 2-14 | 0.30 | 0.83 | 0.06 | 0.009 | 0.0009 | 0.042 | 0.89 | 0.60 | 0.14 | 0.015 | 0.0012 |
| 2-15 | 0.35 | 1.26 | 0.40 | 0.006 | 0.0010 | 0.027 | 0.84 | 0.73 | 0.13 | 0.011 | 0.0014 |
| 2-16 | 0.35 | 0.59 | 0.36 | 0.007 | 0.0010 | 0.055 | 0.70 | 0.60 | 0.08 | 0.011 | 0.0012 |
| 2-17 | 0.47 | 0.42 | 0.15 | 0.012 | 0.0010 | 0.053 | 1.00 | 0.62 | 0.15 | 0.011 | 0.0013 |
| 2-18 | 0.25 | 0.50 | 0.37 | 0.007 | 0.0009 | 0.026 | 1.10 | 1.34 | 0.09 | 0.011 | 0.0015 |
| 2-19 | 0.25 | 0.93 | 0.41 | 0.008 | 0.0010 | 0.033 | 0.70 | 1.15 | 0.17 | 0.013 | 0.0012 |
| 2-20 | 0.30 | 1.23 | 0.36 | 0.007 | 0.0009 | 0.047 | 0.55 | 0.78 | 0.10 | 0.012 | 0.0013 |
| 2-21 | 0.25 | 1.25 | 0.39 | 0.006 | 0.0007 | 0.033 | 0.69 | 0.78 | 0.09 | 0.015 | 0.0014 |
| 2-22 | 0.42 | 0.47 | 0.22 | 0.006 | 0.0009 | 0.027 | 0.02 | 1.17 | 0.11 | 0.013 | 0.0012 |
| 2-23 | 0.30 | 0.44 | 0.35 | 0.007 | 0.0006 | 0.043 | 0.84 | 0.01 | 0.11 | 0.009 | 0.0011 |
| 2-24 | 0.42 | 1.27 | 0.98 | 0.009 | 0.0010 | 0.027 | 0.95 | 0.82 | 0.08 | 0.010 | 0.0015 |
| 2-25 | 0.36 | 1.10 | 0.29 | 0.009 | 0.0010 | 0.038 | 0.63 | 1.10 | 0.11 | 0.011 | 0.0014 |
| 2-26 | 0.43 | 0.70 | 0.36 | 0.057 | 0.0009 | 0.053 | 0.91 | 0.85 | 0.10 | 0.014 | 0.0011 |

### [Table 4-2]

**TABLE 4-2**

| Test Number | Chemical Composition (unit is mass%; balance is Fe and impurities. | | | | | | | | | | |
|---|---|---|---|---|---|---|---|---|---|---|---|
| | N | O | Nb | Ca | Mg | Zr | REM | Co | W | Ni | Cu |
| 2-1 | 0.0043 | 0.0018 | - | - | - | - | - | - | - | - | - |
| 2-2 | 0.0027 | 0.0008 | - | - | - | - | - | - | - | - | - |
| 2-3 | 0.0028 | 0.0013 | - | - | - | - | - | - | - | - | - |
| 2-4 | 0.0022 | 0.0010 | - | - | - | - | - | - | - | - | - |
| 2-5 | 0.0025 | 0.0019 | - | - | - | - | - | - | - | - | - |
| 2-6 | 0.0024 | 0.0010 | 0.013 | - | - | - | - | - | - | - | - |
| 2-7 | 0.0031 | 0.0014 | - | 0.0017 | - | - | - | - | - | - | - |
| 2-8 | 0.0035 | 0.0012 | - | - | 0.0019 | - | - | - | - | - | - |
| 2-9 | 0.0046 | 0.0015 | - | - | - | 0.0013 | - | - | - | - | - |
| 2-10 | 0.0043 | 0.0018 | - | - | - | - | 0.0023 | - | - | - | - |
| 2-11 | 0.0040 | 0.0019 | - | - | - | - | - | 0.31 | - | - | - |
| 2-12 | 0.0028 | 0.0016 | - | - | - | - | - | - | 0.29 | - | - |
| 2-13 | 0.0036 | 0.0008 | - | - | - | - | - | - | - | 0.03 | - |
| 2-14 | 0.0033 | 0.0006 | - | - | - | - | - | - | - | - | 0.22 |
| 2-15 | 0.0040 | 0.0011 | - | - | - | - | - | - | - | - | - |
| 2-16 | 0.0037 | 0.0007 | 0.015 | - | - | - | - | - | - | - | - |
| 2-17 | 0.0025 | 0.0017 | - | - | - | - | - | - | - | - | - |
| 2-18 | 0.0045 | 0.0011 | - | - | - | - | - | - | - | - | - |
| 2-19 | 0.0042 | 0.0017 | - | - | - | - | - | - | - | - | - |
| 2-20 | 0.0047 | 0.0010 | - | - | - | - | - | - | - | - | - |
| 2-21 | 0.0032 | 0.0015 | - | - | - | - | - | - | - | - | - |
| 2-22 | 0.0041 | 0.0014 | - | - | - | - | - | - | - | - | - |
| 2-23 | 0.0039 | 0.0011 | - | - | - | - | - | - | - | - | - |
| 2-24 | 0.0026 | 0.0014 | - | - | - | - | - | - | - | - | - |
| 2-25 | 0.0346 | 0.0015 | - | - | - | - | - | - | - | - | - |
| 2-26 | 0.0031 | 0.0010 | - | - | - | - | - | - | - | - | - |

Ingots were produced using the molten steels of Test Nos. 2-1 to 2-26. The produced ingots were subjected to hot rolling to produce steel plates having a thickness of 15 mm. The steel plates of Test Nos. 2-1 to 2-26 after hot rolling were each allowed to cool to bring the temperature of the steel plate to normal temperature (25°C). After being allowed to cool, the steel plates of Test Nos. 2-1 to 2-26 were held for 20 minutes at the quenching temperature (920°C), and thereafter the steel plates were immersed in a water bath to be quenched. At this time, the cooling rate during quenching (CR₈₀₀₋₅₀₀) was 600°C/min for each test number. Note that, a type K thermocouple of a sheath type was inserted into a center portion of the thickness of the steel plate in advance, and the quenching temperature and cooling rate during quenching CR₈₀₀₋₅₀₀ were measured using the type K thermocouple.

After quenching, the steel plates of Test Nos. 2-1 to 2-26 were subjected to tempering. In the present example, tempering at a high temperature is also referred to as "first tempering", and tempering at an intermediate temperature is also referred to as "second tempering". The holding temperature (°C), holding time (minutes), and diffusion length (√Dt_{H} (nm) or √Dt_{L} (nm)) for the first tempering and the second tempering are shown in Table 5. In addition, the diffusion length √Dt_{To} (nm) in the overall tempering as determined based on the diffusion lengths √Dt_{H} and √Dt_{L} and Formula (8) is shown in Table 5. Note that, in Table 5, the symbol "-" in the column "First Tempering" means that the first tempering was not performed. Similarly, in Table 5, the symbol "-" in the column "Second Tempering" means that the second tempering was not performed.

### [Table 5]

**TABLE 5**

| Test Number | First Tempering | | | Second Tempering | | | Overall Tempering √D_{To} (nm) |
|---|---|---|---|---|---|---|---|
| | Holding Temperature (°C) | Holding Time (min) | √Dt_{H} (nm) | Holding Temperature (°C) | Holding Time (min) | √Dt_{L} (nm) | |
| 2-1 | 700 | 60 | 104.9 | 550 | 900 | 7.0 | 105.1 |
| 2-2 | 710 | 60 | 136.2 | 550 | 900 | 7.0 | 136.4 |
| 2-3 | - | - | - | 550 | 129600 | 84.4 | 84.4 |
| 2-4 | 690 | 60 | 81.0 | 550 | 900 | 7.0 | 81.3 |
| 2-5 | 700 | 60 | 104.9 | 550 | 900 | 7.0 | 105.1 |
| 2-6 | 700 | 60 | 104.9 | 550 | 900 | 7.0 | 105.1 |
| 2-7 | 710 | 40 | 111.2 | 550 | 900 | 7.0 | 111.4 |
| 2-8 | 700 | 80 | 121.1 | 600 | 180 | 13.3 | 121.8 |
| 2-9 | 700 | 60 | 104.9 | 550 | 600 | 5.7 | 105.0 |
| 2-10 | 710 | 60 | 136.2 | 550 | 900 | 7.0 | 136.4 |
| 2-11 | 700 | 80 | 121.1 | 550 | 900 | 7.0 | 121.3 |
| 2-12 | 690 | 70 | 87.4 | 550 | 1200 | 8.1 | 87.8 |
| 2-13 | 705 | 60 | 119.5 | 550 | 500 | 5.2 | 119.6 |
| 2-14 | 690 | 90 | 99.2 | 500 | 2880 | 2.6 | 99.2 |
| 2-15 | 710 | 60 | 136.2 | - | - | - | 136.2 |
| 2-16 | 700 | 60 | 104.9 | - | - | - | 104.9 |
| 2-17 | 700 | 50 | 95.7 | 680 | 30 | 44.3 | 105.5 |
| 2-18 | 680 | 60 | 62.6 | 570 | 40 | 2.7 | 62.7 |
| 2-19 | 690 | 50 | 73.9 | 560 | 80 | 2.8 | 74.0 |
| 2-20 | 680 | 60 | 62.6 | 500 | 80 | 0.4 | 62.6 |
| 2-21 | 680 | 60 | 62.6 | 500 | 180 | 0.7 | 62.6 |
| 2-22 | 700 | 60 | 104.9 | 550 | 900 | 7.0 | 105.1 |
| 2-23 | 680 | 60 | 62.6 | 550 | 900 | 7.0 | 63.0 |
| 2-24 | 710 | 60 | 136.2 | 550 | 900 | 7.0 | 136.4 |
| 2-25 | 700 | 80 | 121.1 | 550 | 900 | 7.0 | 121.3 |
| 2-26 | 700 | 60 | 104.9 | 550 | 900 | 7.0 | 105.1 |

Here, the temperature of the heat treatment furnace where tempering was performed was adopted as the holding temperature during tempering in the present example. In addition, the holding time during tempering in the present example was taken as the time from when the temperature of the steel plate of each test number reached a predetermined tempering temperature until the steel plate was extracted from the heat treatment furnace.

### [Evaluation test]

The steel plates of Test Nos. 2-1 to 2-26 on which tempering had been performed were subjected to a tensile test, a dislocation density measurement test, a grain boundary Mo amount measurement test, and a DCB test that are described hereunder.

### [Tensile test]

The steel plates of Test Nos. 2-1 to 2-26 were subjected to a tensile test by the method described above. Specifically, a round bar tensile test specimen having a parallel portion diameter of 4 mm and a gage length of 16 mm was prepared from a center portion of the thickness of each steel plate of Test Nos. 2-1 to 2-26. The axial direction of the round bar tensile test specimen was parallel to the rolling elongation direction of the steel plate. Using the round bar specimens of Test Nos. 2-1 to 2-26, a tensile test in accordance with ASTM E8/E8M (2021) was carried out at normal temperature (25°C) in the atmosphere, and the yield strength (MPa) of each steel plate of Test Nos. 2-1 to 2-26 was determined. The obtained yield strength is shown as "Yield Strength σ_{YS} (MPa)" in Table 6.

### [Table 6]

**TABLE 6**

| Test Number | Yield Strength σ_{YS} (MPa) | Dislocation Density ρ (10¹⁴ m⁻²) | Grain Boundary Mo Amount γ_{Mo} (mass%) | Fn1 | K_{1SSC} (MPa√m) |
|---|---|---|---|---|---|
| 2-1 | 901 | 10.2 | 10.1 | -328 | 28.0 |
| 2-2 | 915 | 7.8 | 10.6 | -267 | 28.3 |
| 2-3 | 867 | 8.7 | 19.3 | 490 | 29.8 |
| 2-4 | 890 | 8.8 | 8.9 | -398 | 26.5 |
| 2-5 | 879 | 7.8 | 10.8 | -214 | 28.7 |
| 2-6 | 896 | 8.1 | 9.7 | -327 | 27.7 |
| 2-7 | 883 | 8.1 | 9.3 | -347 | 27.4 |
| 2-8 | 879 | 8.5 | 15.3 | 149 | 29.4 |
| 2-9 | 890 | 9.0 | 9.4 | -359 | 27.3 |
| 2-10 | 873 | 8.5 | 10.4 | -252 | 28.9 |
| 2-11 | 864 | 8.5 | 10.7 | -218 | 29.0 |
| 2-12 | 906 | 10.8 | 11.5 | -224 | 28.6 |
| 2-13 | 876 | 7.2 | 8.5 | -393 | 26.7 |
| 2-14 | 900 | 9.8 | 8.0 | -496 | 24.6 |
| 2-15 | 878 | 13.2 | 5.6 | -715 | 22.8 |
| 2-16 | 889 | 13.6 | 5.3 | -755 | 22.6 |
| 2-17 | 913 | 12.3 | 5.9 | -714 | 23.4 |
| 2-18 | 932 | 12.4 | 8.3 | -535 | 23.5 |
| 2-19 | 906 | 14.8 | 8.3 | -536 | 23.6 |
| 2-20 | 949 | 12.6 | 5.5 | -787 | 22.9 |
| 2-21 | 927 | 10.2 | 5.6 | -727 | 23.0 |
| 2-22 | 904 | 8.0 | 9.5 | -350 | 16.0 |
| 2-23 | 909 | 10.2 | 0.0 | -1174 | 15.2 |
| 2-24 | 903 | 8.0 | 8.9 | -399 | 11.3 |
| 2-25 | 898 | 8.7 | 9.4 | -363 | 17.4 |
| 2-26 | 928 | 8.5 | 8.9 | -431 | 10.9 |

### [Dislocation density measurement test]

The steel plates of Test Nos. 2-1 to 2-26 were subjected to a dislocation density measurement test by the method described above. Specifically, a test specimen of 20 mm in width × 20 mm in length × 2 mm in thickness was prepared from a center portion of the thickness of each steel plate of Test Nos. 2-1 to 2-26. The half-value width ΔK of the peaks of the (110), (211), and (220) planes was determined using X-ray diffraction according to the method described above. The determined half-value widths ΔK were used to determine the dislocation density ρ (m⁻²) by the method described above. The obtained dislocation density is shown as "Dislocation Density ρ (10¹⁴ m⁻²)" in Table 6.

### [Grain boundary Mo amount measurement test]

The steel plates of Test Nos. 2-1 to 2-26 were subjected to a grain boundary Mo amount measurement test by the method described above. Specifically, for each of the steel plates of Test Nos. 2-1 to 2-26, a test specimen was prepared which included a thickness t/4 position at the center thereof and which had a size having a length of 10 mm in the rolling elongation direction × 5 mm in the width direction × 8 mm in the thickness direction. The prepared test specimen was used to obtain the grain boundary Mo amount (mass%) by the method described above. The obtained grain boundary Mo amount is shown as "Grain Boundary Mo Amount γ_{Mo} (mass%)" in Table 6. In addition, Fnl was obtained using the obtained yield strength σ_{YS} (MPa), dislocation density ρ (m⁻²), and grain boundary Mo amount γ_{Mo} (mass%), and Formula (1). The obtained Fn1 is shown in Table 6.

### [DCB test]

The steel plates of Test Nos. 2-1 to 2-26 were subjected to a DCB test by the method described above. Specifically, a DCB test specimen and a wedge that are described above were prepared from a center portion of the thickness of each of the steel plates of Test Nos. 2-1 to 2-26. A DCB test in accordance with NACE TM0177-2016 Method D was performed under the conditions described above using the prepared test specimen and wedge. The fracture toughness value K_{1SSC} obtained by the DCB test performed by the method described above is shown as "K_{1SSC} (MPa√m)" in Table 6.

### [Evaluation results]

Referring to Table 4-1, Table 4-2, Table 5, and Table 6, in each of the steel plates of Test Nos. 2-1 to 2-14, the chemical composition was appropriate and the yield strength was 862 MPa or more (125 ksi or more). In addition, the grain boundary Mo amount γ_{Mo} was 5.0% by mass or more, and Fn1 was -520 or more. As a result, the K_{1SSC} value was 24.1 MPa or more. That is, these steel plates had a yield strength of 110 ksi or more, and had excellent fracture toughness in a low-temperature sour environment.

On the other hand, the steel plates of Test Nos. 2-15 and 2-16 were not subjected to an intermediate-temperature tempering process. As a result, for these steel plates, Fnl was less than -520. Consequently, the K_{1SSC} value of each of these steel plates was less than 24.1 MPa. That is, these steel plates did not have excellent fracture toughness in a low-temperature sour environment.

For the steel plate of Test No. 2-17, in the intermediate-temperature tempering process, the holding temperature was too high and the holding time was too short. As a result, for this steel plate, Fnl was less than -520. Consequently, the K_{1SSC} value of this steel plate was less than 24.1 MPa. That is, this steel plate did not have excellent fracture toughness in a low-temperature sour environment.

For the steel plates of Test Nos. 2-18 and 2-19, the holding time in the intermediate-temperature tempering process was too short. As a result, for these steel plates, Fnl was less than -520. Consequently, the K_{1SSC} value for each of these steel plates was less than 24.1 MPa. That is, these steel plates did not have excellent fracture toughness in a low-temperature sour environment.

For the steel plate of Test No. 2-20, in the intermediate-temperature tempering process, the holding time was too short and the diffusion length √Dt_{L} was too small. As a result, for this steel plate, Fnl was less than -520. Consequently, the K_{1SSC} value of this steel plate was less than 24.1 MPa. That is, this steel plate did not have excellent fracture toughness in a low-temperature sour environment.

For the steel plate of Test No. 2-21, the diffusion length √Dt_{L} in the intermediate-temperature tempering process was too small. As a result, for this steel plate, Fnl was less than -520. Consequently, the K_{1SSC} value of this steel plate was less than 24.1 MPa. That is, this steel plate did not have excellent fracture toughness in a low-temperature sour environment.

In the steel plate of Test No. 2-22, the content of Cr was too low. As a result, the K_{1SSC} value of this steel plate was less than 24.1 MPa. That is, this steel plate did not have excellent fracture toughness in a low-temperature sour environment.

In the steel plate of Test No. 2-23, the content of Mo was too low. As a result, in this steel plate, the grain boundary Mo amount γ_{Mo} was less than 5.0% by mass, and Fnl was less than -520. Consequently, the K_{1SSC} value of this steel plate was less than 24.1 MPa. That is, this steel plate did not have excellent fracture toughness in a low-temperature sour environment.

In the steel plate of Test No. 2-24, the content of Mn was too high. As a result, the K_{1SSC} value of this steel plate was less than 24.1 MPa. That is, this steel plate did not have excellent fracture toughness in a low-temperature sour environment.

In the steel plate of Test No. 2-25, the content of N was too high. As a result, the K_{1SSC} value of this steel plate was less than 24.1 MPa. That is, this steel plate did not have excellent fracture toughness in a low-temperature sour environment.

In the steel plate of Test No. 2-26, the content of P was too high. As a result, the K_{1SSC} value of this steel plate was less than 24.1 MPa. That is, this steel plate did not have excellent fracture toughness in a low-temperature sour environment.

An embodiment of the present disclosure has been described above. However, the embodiment described above is merely an example for carrying out the present disclosure. Therefore, the present disclosure is not limited to the above-described embodiment, and can be implemented by appropriately modifying the above-described embodiment within a range not departing from the spirit thereof.

## Claims

1. A steel material consisting of, in mass%,
C: more than 0.20 to 0.60%,
Si: 0.05 to 2.00%,
Mn: 0.02 to 0.60%,
P: 0.025% or less,
S: 0.0100% or less,
Al: 0.005 to 0.100%,
Cr: 0.20 to 1.50%,
Mo: 0.35 to 1.50%,
V: 0.01 to 0.60%,
Ti: 0.002 to 0.050%,
B: 0.0001 to 0.0050%,
N: 0.0100% or less,
O: 0.0100% or less,
Nb: 0 to 0.030%,
Ca: 0 to 0.0100%,
Mg: 0 to 0.0100%,
Zr: 0 to 0.0100%,
rare earth metal: 0 to 0.0100%,
Co: 0 to 0.50%,
W: 0 to 0.50%,
Ni: 0 to 0.20%, and
Cu: 0 to 0.50%,
with the balance being Fe and impurities;
wherein:
a yield strength σ_{YS} is 758 MPa or more;
in the steel material, a content of Mo near prior-austenite grain boundaries γ_{Mo} is 5.0% by mass or more;
in a case where the yield strength σ_{YS} is less than 862 MPa, Fnl defined by Formula (1) satisfies -300 or more; and
in a case where the yield strength σ_{YS} is 862 MPa or more, Fnl defined by Formula (1) satisfies -520 or more; $Fn 1 = 83 \times \left({γ}_{Mo}-{10}^{- 7}\times √ρ\right) - {σ}_{YS}$
where, the content of Mo near prior-austenite grain boundaries in percent by mass is substituted for γ_{Mo} in Formula (1), a dislocation density in m⁻² is substituted for ρ in Formula (1), and the yield strength in MPa is substituted for σ_{YS} in Formula (1).

2. The steel material according to claim 1, containing one or more elements selected from a group consisting of:
Nb: 0.001 to 0.030%,
Ca: 0.0001 to 0.0100%,
Mg: 0.0001 to 0.0100%,
Zr: 0.0001 to 0.0100%,
rare earth metal: 0.0001 to 0.0100%,
Co: 0.01 to 0.50%,
W: 0.01 to 0.50%,
Ni: 0.01 to 0.20%, and
Cu: 0.01 to 0.50%.

3. The steel material according to claim 1 or claim 2, wherein:
the steel material is an oil-well steel pipe.
